



US005354642A

**United States Patent [19]****Texter et al.****Patent Number: 5,354,642****Date of Patent: \* Oct. 11, 1994****[54] POLYMERIC COUPLERS FOR HEAT IMAGE SEPARATION SYSTEMS****[75] Inventors:** **John Texter, Rochester; Tienteh Chen, Penfield; Ronald H. White, Rochester, all of N.Y.****[73] Assignee:** **Eastman Kodak Company, Rochester, N.Y.****[\*] Notice:** The portion of the term of this patent subsequent to Dec. 14, 2010 has been disclaimed.**[21] Appl. No.:** **927,691****[22] Filed:** **Aug. 10, 1992****[51] Int. Cl.<sup>5</sup>** **..... G03C 5/54; G03C 7/32****[52] U.S. Cl.** **..... 430/203; 430/351; 430/548; 430/226****[58] Field of Search** **..... 430/203, 226, 201, 199, 430/548****[56] References Cited****U.S. PATENT DOCUMENTS**

- 3,926,436 12/1975 Monbaliu et al. .  
 4,080,211 3/1978 Van Paesschen et al. .  
 4,215,195 7/1980 Ponticello et al. .  
 4,455,363 6/1984 Naito et al. .... 430/548  
 4,474,870 10/1984 Yagihara et al. .  
 4,511,647 4/1985 Hirano et al. .  
 4,518,687 5/1985 Hirano et al. .  
 4,522,916 6/1985 Hirano .  
 4,576,910 3/1986 Hirano et al. .  
 4,612,278 9/1986 Lau et al. .  
 4,631,251 12/1986 Komamura et al. .... 430/226  
 4,650,748 3/1987 Komamura et al. .... 430/226  
 4,656,124 4/1987 Komamura .... 430/548  
 4,756,998 7/1988 Helling et al. .  
 4,847,188 7/1989 Komamura et al. .... 430/203  
 4,874,689 10/1989 Yamanouchi et al. .  
 4,921,782 5/1990 Helling .  
 4,946,771 8/1990 Maekawa et al. .  
 5,032,499 7/1991 Kohno et al. .... 430/203  
 5,164,280 11/1992 Texter et al. .... 430/235  
 5,270,145 12/1993 Willis et al. .... 430/203

**FOREIGN PATENT DOCUMENTS**

- 0283938A1 9/1988 European Pat. Off. .  
 0316955A3 5/1989 European Pat. Off. .  
 0321399A3 6/1989 European Pat. Off. .  
 0259864B1 9/1991 European Pat. Off. .  
 4-73751 3/1992 Japan .  
 2092573B 10/1984 United Kingdom .

**Primary Examiner—Richard L. Schilling  
Attorney, Agent, or Firm—Paul A. Leipold****[57] ABSTRACT****A process is disclosed for forming a dye image including the steps of:****exposing a photographic element comprising a support bearing a light sensitive silver halide emulsion layer containing a polymeric color coupler compound capable of forming a heat transferable dye upon development, wherein the polymeric color coupler compound is of the formula:****COUP-L-B**

wherein COUP represents a coupler moiety capable of forming a heat transferable dye upon reaction of the moiety with an oxidation product of a color developer; L is a divalent linking group which is separated from COUP upon reaction of the coupler moiety with said oxidation product of a color developer; and B represents the polymeric backbone;  
 developing said exposed element with a color developer solution to form a heat transferable dye image; heating said exposed, developed element to thereby transfer the dye image from the emulsion layer to a dye receiving layer, where said receiving layer is part of the photographic element or part of a separate dye receiving element brought into contact with the photographic element; and  
 separating the emulsion layer from the dye receiving layer containing the transferred dye image.

**53 Claims, 3 Drawing Sheets**



FIG. 1



FIG. 2



FIG. 3



FIG. 4



FIG. 5

## POLYMERIC COUPLERS FOR HEAT IMAGE SEPARATION SYSTEMS

This invention is related to copending, commonly assigned U.S. application Ser. No. 7/804,877, filed Dec. 6, 1991, *Heat Image Separation System* of Willis and Texter now U.S. Pat. No. 5,270,145, to U.S. application Ser. No. 7/804,868, filed Dec. 6, 1991, *Thermal Solvents for Dye Diffusion in Image Separation Systems* of Bailey et al., and to U.S. application Ser. No. 7/805,717, filed Dec. 6, 1991, *Mechanicochemical Layer Stripping in Image Separation Systems* of Texter et al, now U.S. Pat. No. 5,164,280.

### TECHNICAL FIELD

This invention relates to photographic systems and processes for forming a dye image in a light sensitive silver halide emulsion layer, and subsequently separating the dye image from the emulsion layer. More particularly, this invention relates to wet development processes for forming dye images in silver halide emulsion layers and to thermal dye diffusion image separation systems.

### BACKGROUND INFORMATION

#### Wet Development—Dry Thermal Transfer Systems

In conventional "wet" silver halide based color photographic processing systems, an imagewise exposed photographic element, for example color paper designed to provide color prints, is processed in a color developer solution. The developer reduces the exposed silver halide of the photographic element to metallic silver and the resulting oxidized developer reacts with incorporated dye-forming couplers to yield dye images corresponding to the imagewise exposure. As silver is generally grey and desaturates the pure colors of the dyes, it is desirable to remove it from the dye images. Silver is conventionally separated from the dye images by a process of bleaching the silver to a silver halide and removing the silver halide by using an aqueous solvent, a fixing bath. This fixing bath also removes the undeveloped original silver halide. Commonly, the bleach and fix are combined into one solution, a bleach-fix solution.

Bleach-fix solutions commonly contain iron, ammonium, ethylenediaminetetraacetic acid, thiosulfate and, after use, silver. These components of "wet" silver halide processing are the source of much of the pollution from photo finishing processes. "Dry" silver halide based color photographic processing systems have been proposed which employ thermally developable color photographic material. Such thermally developable materials generally comprise a light sensitive layer containing silver halide, a photographic coupler or other dye-providing material, and a color developing agent as disclosed, e.g., in U. Pat. Nos. 4,584,267 and 4,948,698 and references cited therein. After image-wise exposure, these elements can be developed by uniformly heating the element to activate the developing agent incorporated therein, thereby eliminating the need for wet processing with a developer solution. In some thermally developable systems, the dye-providing materials are designed to form diffusible dyes upon heat development, which may be transferred to an image-receiving layer either during thermal development or thereafter in a separate step. Such thermally developable diffusion transfer color photography systems are disclosed in U. Pat. Nos. 4,584,267 and 4,948,698 referenced above.

These systems also eliminate the need for bleach-fix steps with processing solutions and the resulting effluent wastes.

### Polymeric Couplers

It is also known in the art that couplers may be incorporated in the form of a polymer which improves the ability of the dye to remain in the location where it is formed in a color photographic element. For example, 10 Monbaliu et al. disclose (U.S. Pat. No. 3,926,436) photographic elements containing polymeric couplers as latexes which show less foaming tendency and which show high compatibility with hydrophilic colloids such as gelatin. Yagihara et al. (U.S. Pat. No. 4,474,870) disclose photographic materials containing polymeric coupler latexes that form magenta dyes upon coupling with oxidized developing agents. Hirano et al. (U.S. Pat. No. 4,511,647) disclose color photographic materials containing cyan color forming coupler latexes. 20 Yagihara et al. (U.K. Pat. No. 2,092,573 B) disclose silver halide photographic materials containing magenta color forming coupler latexes. Cawse and Harris (European Pat. Application 0321399 A3) disclose a method of preparing latexes of color couplers.

25 Generally, three methods have been employed in the past for dispersing polymeric couplers. These three methods include: (1) dispersing the coupler by colloid milling or homogenization methods, along with high and/or low vapor pressure organic solvents in aqueous surfactant and gelatin; (2) direct incorporation of solutions of water soluble polymers; (3) latex formation by emulsion polymerization or suspension polymerization.

30 Hirano (U.S. Pat. No. 4,522,916) discloses the preparation of polymeric magenta dye forming coupler latexes that provide images of improved light stability. Hirano discloses a series of magenta dye forming coupler monomers, wherein the coupling moieties are attached to the ethylenic group through a linking group attached to the coupling site. Hirano and Furutachi (U.S. Pat. No. 4,576,910) disclose the preparation of 35 polymeric magenta dye forming coupler latexes formed from triazole and tetrazole monomers. Helling et al. (U.S. Pat. No. 4,756,998) disclose the preparation of 40 polymeric couplers which contain at least one urethane or urea group. Yamanouchi et al. (U.S. Pat. No. 4,874,689) disclose the preparation of polymeric couplers utilizing chain transfer agents of eight or more carbon atoms, and wherein the coupling moieties are 45 attached to the ethylenic group through a linking group attached at the coupling site. Helling (U.S. Pat. No. 4,921,782) discloses the preparation of polymeric magenta dye forming couplers, wherein the magenta coupler monomer contains a carboxyl group. Maekawa and Hirano (U.S. Pat. No. 4,946,771) disclose the preparation of 50 polymeric couplers formulated with certain advantageously incorporated coupling and noncoupling comonomers.

55 Sakanoue and Hirano (European Patent Application 0 259 864 A2) disclose the preparation of water-soluble yellow dye-forming polymeric couplers containing a repeating unit derived from at least one monomer in which the polymerization moiety is in a coupling-off group. Yamanouchi et al. (European Patent Application 0 316 955 A3) disclose several ethylenic coupling monomers wherein the coupling moieties are attached to the 60 ethylenic group through a linking group attached to the coupling site. Hirano et al. (European Patent Application 0 316 955 A3) disclose several ethylenic coupling monomers wherein the coupling moieties are attached to the 65 ethylenic group through a linking group attached to the coupling site. Hirano et al. (European Patent Application

tion 0 283 938 A1) disclose polymeric couplers wherein the coupling moieties are attached to the polymeric backbone through linking groups that are attached to the coupling site.

Polymeric couplers can be prepared by joining reactive couplers to synthesized polymers. Such polymers may include polyacrylic acid, poly-p-aminostyrene, and other natural high polymers. Methods for producing such polymeric couplers are described in U.S. Pat. Nos. 2,698,797, 2,852,381, 2,852,383, and 2,870,712 and in Japanese Patent Publication Nos. 16932/1960 and 3661/1969. Methods for forming polymeric couplers from ethylenically unsaturated monomers and other polymerizable monomers are disclosed in British Pat. Nos. 880,206, 955,197, 967,503, 967,504, 995,363, and 1,104,658.

Jones disclosed (U.S. Pat. No. 2,561,205) the formation of water-soluble polymeric couplers derived from  $\beta,\gamma$ -ethylenically unsaturated amides. Williams disclosed (U.S. Pat. No. 2,739,956) the formation of water-soluble polymeric couplers derived from vinyl-substituted monomers such as 2-vinyl-1-naphthol. Firestine disclosed (U.S. Pat. No. 2,976,294) water-soluble polymers derived from methacrylamide related monomers, such as 1-(m-methacryloylaminophenyl)-2-carboxy-5-pyrazolone.

Umberger (U.S. Pat. No. 3,451,820) discloses dispersions of lipophilic colorforming polymeric couplers. Van Paesschen and Priem (U.S. Pat. No. 4,080,211) disclose a process for making color-coupling agents by emulsion polymerization. Ponticello et al. (U.S. Pat. No. 4,215,195) disclose the preparation of cross-linkable polymers that contain color-forming coupler residues. Hirano et al. (U.S. Pat. No. 4,518,687) disclose a photographic material containing a cyan dye-forming oleophilic polymeric coupler. Lau and Tang (U.S. Pat. No. 4,612,278) disclose photographic materials containing polymeric couplers copolymerized with alkoxyalkylacrylate monomers.

#### Problems

While dry processing systems as discussed above are beneficial in that they eliminate the need for processing solutions and the resulting waste, they require additional materials, such as developing agents, to be incorporated into the thermally developable photographic element itself. Also, the levels of silver halide necessary for heat developable systems are generally substantially higher than those required for conventional wet systems. The presence of such additional materials can detrimentally affect the cost, performance, and storage properties of such elements.

It would be desirable to provide a photographic processing system which would reduce the amount of waste processing solution effluents generated by the overall processing system while retaining the benefits of image quality and industry compatibility which are derived from wet development with conventional developing solutions.

A previously unrecognized problem in wet development/dry thermal transfer systems is that considerable quantities of coupler are routinely transferred to the receiver in addition to the dye. This thermal transfer of coupler is unwanted and undesirable because unwanted hue effects can result, the transferred coupler can result in unwanted printout as the result of chemical transformations of the transferred coupler, and the thermally transferred coupler can cause difficult to control anom-

alies in the thermal stability of the transferred dye and the glass transition temperature of the receiver element.

These and other problems may be overcome by the practice of our invention.

#### SUMMARY OF THE INVENTION

An object of the invention is to overcome disadvantages of prior processes. Another object of the invention is to provide dye images of improved hue. Yet another object is to provide heat transferable dyes while reducing or eliminating the presence of heat transferable coupling moieties. A further object is to provide improved coupling reactivity.

An object of the present invention is to provide coating melts of improved coatability. Another object is to provide photographic elements of increased storage stability. Yet another object is to provide a process for imaging that utilizes reduced quantities of noxious organic solvents in the dispersal of coupling moieties and to reduce the amount of organic solvents vented to the environment.

These and other objects of the invention are generally achieved by providing a process for forming a dye image comprising the steps of:

exposing a photographic element comprising a support bearing a light sensitive silver halide emulsion layer containing a polymeric color coupler compound capable of forming a heat transferable dye upon development, wherein the polymeric color coupler compound is of the formula:

#### COUP-L-B

wherein COUP represents a coupler moiety capable of forming a heat transferable dye upon reaction of the moiety with an oxidation product of a color developer; L is a divalent linking group which is separated from COUP upon reaction of the coupler moiety with said oxidation product of a color developer; and B represents the polymeric backbone;

developing said exposed element with a color developer solution to form a heat transferable dye image;

heating said exposed, developed element to thereby transfer the dye image from the emulsion layer to a dye receiving layer, where said receiving layer is part of the photographic element or part of a separate dye receiving element brought into contact with the photographic element; and

separating the emulsion layer from the dye receiving layer containing the transferred dye image.

#### BRIEF DESCRIPTION OF THE DRAWINGS

FIG. 1. Status A reflectance densitometry for test receiver elements obtained for the comparison coupler Y3 (curve 1) and for the polymeric coupler Y2 (curve 2) of the present invention.

FIG. 2. Reflection spectra of dye thermally transferred to receiver for coatings of Examples 1 (curve 1 for dye obtained from polymeric coupler Y2) and 2 (curve 2 for dye obtained from conventional coupler Y4).

FIG. 3. Status A reflectance densitometry of test receiver elements obtained for the polymeric coupler Y4 (curve 1) of the present invention and for the comparison coupler Y3 (curve 2).

FIG. 4. Status A reflectance densitometry of test receiver elements obtained for the polymeric coupler

C2 (curve 1) of the present invention and for the comparison coupler C3 (curve 2).

FIG. 5. Reflectance spectra of dye thermally transferred to receiver for coatings of dye obtained from polymeric coupler C2 (curve 1) and from conventional coupler C3 (curve 2).

#### DETAILED DESCRIPTION OF THE INVENTION

While polymeric couplers are now well known in photographic applications, elements, and processes, their general use in the present invention is disadvantageous with respect to the formation of useful diffusion transfer dye images. This disadvantage stems from the fact that most polymeric couplers that have been disclosed react with the oxidation product of primary amine developing agents to produce image dyes, wherein said image dyes are not diffusible. This nondiffusibility stems from the basic nondiffusibility of the polymeric coupler, wherein said coupling moieties are usually attached to the polymeric backbone through a linking group that is not associated with the coupling site of the coupling moiety. Dyes which are formed by conventional color development and subsequent coupling chemistry remain attached to the polymeric backbone, and are therefore nondiffusible and unavailable for color diffusion transfer. However, an entirely different situation obtains for that class of polymeric couplers disclosed in the present invention, wherein said polymeric couplers comprise coupling moieties attached to the polymeric backbone through linking groups, wherein said linking groups are attached to the respective coupling sites. This subclass of polymeric couplers produces diffusible dyes upon reaction with the oxidation product of primary amine developing agents. Said dye-forming reactions sever the coupling moiety from the polymeric backbone.

Accordingly, the use of this special class of polymeric couplers affords numerous advantages in heat image separation systems as described herein. A particularly useful advantage is that the desired image dyes are formed and free to diffuse to receiver elements, while the coupler moieties that do not react to form dye remain nondiffusible. This separation of diffusibilities keeps coupler moieties out of the receiver elements and prevents dye hues from being influenced by the undesired transfer of coupler moieties. This use of polymeric couplers also results in advantageously improved coupling reactivity in many cases, wherein said improvements comprise obtaining higher dye densities. The use of polymeric couplers also results in coating melts with improved coatability; layers containing such polymeric couplers may be coated with less binder, which results in thinner layers, improved sharpness, and improved dye transfer efficiency. The use of polymeric couplers also results in improved storage stability of the coated photographic elements. This storage advantage obtains since conventional coupler dispersions, subject to crystallization as a result of thermodynamic metastability during storage, are replaced by polymeric couplers which cannot crystallize during storage. A further advantage from the use of the polymeric couplers of the present inventions is that the overall use of organic solvents in the dispersal of coupling moieties is reduced. Such solvents such as ethylacetate, cyclohexanone, and the like are routinely used in preparing conventional coupler dispersions for photographic elements, and they must be removed from said dispersions during

manufacture of the elements. Said handling of said solvents imposes unwanted costs and unwanted operator exposure during manufacture. Such handling and exposure is largely eliminated by replacing such conventional coupler dispersions with the polymeric couplers of the present invention.

The coupler moiety of the polymeric coupler of formula (I) which is to be contained in the color photographic material to be used in the process of the invention is designed to be developable by conventional color developer solutions, and to form a heat transferable dye upon such conventional development. While color images may be formed with coupler compounds which form dyes of essentially any hue, couplers which form heat transferable cyan, magenta, or yellow dyes upon reaction with oxidized color developing agents are used in preferred embodiments of the invention.

COUP may represent a coupler moiety, capable of forming a cyan dye by coupling with an aromatic primary amine developing agent. Couplers which form cyan dyes upon reaction with oxidized color developing agents are described in such representative patents as U. Pat. Nos. 2,474,293, 2,772,162, 2,801,171, 2,895,826, 3,002,836, 3,419,390, 3,476,565, 3,779,763, 3,996,252, 4,124,396, 4,248,962, 4,254,212, 4,296,200, 4,333,999, 4,443,536, 4,457,559, 4,500,635, 4,526,864, and 4,874,689 and in European Patent Application No. 0 283 938 A1, the disclosures of which are incorporated by reference. Preferred coupler moieties COUP which form cyan dyes upon reaction with oxidized color developing agents are of the phenol type (formula C-I) or the naphthol type (formulae C-II and C-III) or of the type C-IV; the asterisk mark indicates the position of the bond to the divalent linking group L in formula (I)



In formulae C-I, C-II, C-III, and C-IV above:

$R_1$  has 0 to 30 carbon atoms and represents a possible substituent on the phenol ring or naphthol ring. It is an alkyl group, an alkenyl group, an alkoxy group, an alkoxy carbonyl group, a halogen atom, an alkoxy carbamoyl group, an aliphatic amido group, an alkylsulfonyl group, an alkylsulfonamido group, an alkylureido group, an arylcarbamoyl group, an arylamido group, an arylsulfamoyl group, an arylsulfonamido group, an arylureido group, hydroxyl group, amino group, carboxyl group, sulfo group, heterocyclic group, carbonamido group, sulfonamido group, carbamoyl group, sulfamoyl group, ureido group, acyloxy group, aliphatic oxy group, aliphatic thio group, aliphatic sulfonyl group, aromatic oxy group, aromatic thio group, aromatic sulfonyl group, sulfamoyl amino group, nitro group, or imido group.

$R_2$  represents  $-\text{CONR}_3\text{R}_4$ ,  $-\text{NHCOR}_3$ ,  $-\text{NHCOOR}_5$ ,  $\text{NHSO}_2\text{R}_5$ ,  $-\text{NHCONR}_3\text{R}_4$ , or  $\text{NHSO}_2\text{R}_3\text{R}_4$ ,  $R_3$  and  $R_4$  each represent a hydrogen atom, aliphatic group having 1 to 30 carbon atoms (such as methyl, ethyl, butyl, methoxyethyl, n-decyl, n-dodecyl, n-hexadecyl, trifluoromethyl, heptafluoropropyl, dodecyloxypropyl, 2,4-di-*t*-amylphenoxypropyl, and 2,4-di-*t*-amylphenoxybutyl), aromatic group having from 6 to 30 carbon atoms (such as phenyl, tolyl, 2-tetradecyloxyphenyl, pentafluorophenyl, and 2-chloro-5-dodecyloxy carbonylphenyl), or heterocyclic group having from 2 to 30 carbon atoms (such as 2-pyridyl, 4-pyridyl, 2-furyl, and 2-thienyl).  $R_5$  represents an aliphatic group having from 1 to 30 carbon atoms (such as methyl, ethyl, butyl, methoxyethyl, n-decyl, n-dodecyl, and n-hexadecyl), aromatic group having from 6 to 30 carbon atoms (such as phenyl, tolyl, 4-chlorophenyl, and naphthyl), or heterocyclic group (such as 2-pyridyl, 4-pyridyl, and 2-furyl).  $R_3$  and  $R_4$  may join each other to form a heterocyclic ring (such as morpholine ring, piperidine ring, and pyrrolidine ring);  $p$  is an integer from 0 to 3;  $q$  and  $r$  are integers from 0 to 4;  $s$  is an integer from 0 to 2.

$X_1$  represents an oxygen atom, sulfur atom, or  $R_6\text{N}^<$  group, where  $R_6$  represents a hydrogen atom or monovalent group. When  $R_6$  represents a monovalent group, it includes, for example, an aliphatic group having from 1 to 30 carbon atoms (such as methyl, ethyl, butyl, methoxyethyl, and benzyl), aromatic group having from 6 to 30 carbon atoms (such as phenyl and tolyl), heterocyclic group having from 2 to 30 carbon atoms (such as 2-pyridyl and 2-pyrimidyl), carbonamido group having from 1 to 30 carbon atoms (such as formamido, acetamido, N-methylacetamido, toluenesulfonamido, and 4-chlorobenzenesulfonamido), imido group having from 4 to 30 carbon atoms (such as succinimido),  $-\text{OR}_7$ ,  $-\text{SR}_7$ ,  $-\text{COR}_7$ ,  $-\text{CONR}_7\text{R}_8$ ,  $-\text{COCOR}_7$ ,  $-\text{COCOR}_7\text{R}_8$ ,  $-\text{COOR}_7$ ,  $-\text{COCOOR}_9$ ,  $-\text{SO}_2\text{R}_9$ ,  $-\text{SO}_2\text{OR}_9$ ,  $-\text{SO}_2\text{NR}_7\text{R}_8$ , or  $-\text{NR}_7\text{R}_8$ .  $R_7$  and  $R_8$ , which may be the same or different, each represent a hydrogen atom, aliphatic group having from 1 to 30 carbon atoms (such as methyl, ethyl, butyl, methoxyethyl, n-decyl, n-dodecyl, n-hexadecyl, trifluoromethyl, heptafluoropropyl, dodecyloxypropyl, 2,4-di-*t*-amylphenoxypropyl, and 2,4-di-*t*-amylphenoxybutyl), aromatic group having from 6 to 30 carbon atoms (such as phenyl, tolyl, 2-tetradecyloxyphenyl, pentafluorophenyl, and 2-chloro-5-dodecyloxy carbonylphenyl), or heterocyclic group having from 2 to 30 carbon atoms (such as 2-pyridyl, 4-pyridyl, 2-furyl, and 2-thienyl).  $R_7$  and  $R_8$  may join each other to form a heterocyclic ring (such as morpholine group and piperidino group).  $R_9$

may include, for example, those substituents (excluding a hydrogen atom) exemplified for  $R_7$  and  $R_8$ .

$T$  represents a group of atoms required to form a 5-, 6-, or 7-membered ring by connecting with the carbon atoms. It represents, for example



or a combination thereof. In the formulae above,  $\text{R}'$  and  $\text{R}''$  each represent a hydrogen atom, alkyl group, aryl group, halogen atom, alkoxy group, alkoxy carbonyl group, aryl carbonyl group, alkyl carbamoyl group, aryl carbamoyl group or cyano group.

The preferred substituent groups in the present invention are exemplified in the following:

$R_1$  includes a halogen atom (such as fluorine, chlorine, and bromine), aliphatic group (such as methyl, ethyl, and isopropyl), carbonamido group (such as acetamido and benzamido), and sulfonamido (such as methanesulfonamido and toluenesulfonamido).

$R_2$  includes  $-\text{CONR}_3\text{R}_4$  (such as carbamoyl, ethyl carbamoyl, morpholinocarbonyl, dodecyl carbamoyl, hexadecyl carbamoyl, decyloxypropyl, dodecyloxypropyl, 2,4-di-*t*-amylphenoxypropyl, and 2,4-di-*t*-amylphenoxybutyl).  $X_1$  includes  $\text{R}_6\text{N}^<$ , wherein  $\text{R}_6$  is preferably  $-\text{COR}_7$  (such as formyl, acetyl, trifluoroacetyl, benzoyl, pentafluorobenzoyl, and p-chlorobenzoyl),  $-\text{COOR}_9$  (such as methoxycarbonyl, ethoxycarbonyl, butoxycarbonyl, dodecyloxy carbonyl, methoxyethoxy carbonyl, and phenoxy carbonyl),  $-\text{SO}_2\text{R}_9$  (such as methanesulfonyl, ethanesulfonyl, butanesulfonyl, hexadecanesulfonyl, benzenesulfonyl, toluenesulfonyl, and p-chlorobenzenesulfonyl),  $-\text{CONR}_7\text{R}_8$  (such as N,N-dimethyl carbamoyl, N,N-diethyl carbamoyl, N,N-dimethyl carbamoyl, N,N-diethyl carbamoyl, N,N-dibutyl carbamoyl, morpholinocarbonyl, piperidinocarbonyl, 4-cyanophenyl carbamoyl, 3,4-dichlorophenyl carbamoyl, and 4-methanesulfonylphenyl carbamoyl, and N,N-dibutyl carbamoyl), and  $-\text{SO}_2\text{NR}_7\text{R}_8$  (such as N,N-dimethylsulfamoyl, N,N-diethylsulfamoyl, and N,N-dipropylsulfamoyl). Particularly preferred examples of  $\text{R}_6$  are those groups represented by  $-\text{COR}_7$ ,  $-\text{COOR}_9$ , and  $-\text{SO}_2\text{R}_9$ .

$R_1$  may be substituted. Preferred substituents are aryl groups (such as phenyl), nitro group, hydroxy group, cyano group, sulfo group, an alkoxy group (such as methoxy), an aryloxy group (such as phenoxy), an acyloxy group (such as acetoxy), an acylamino group (such as acetyl amino), an alkylsulfonamido group (such as methanesulfonamido), an alkylsulfamoyl group (such as fluorine atom, chlorine atom, bromine atom), carboxyl group, an alkyl carbamoyl group (such as methyl carbamoyl), an alkoxy carbonyl group (such as methoxy carbonyl), an alkylsulfonyl group (such as methysulfonyl), an alkylthio group (such as  $\beta$ -carboxyethylthio), etc. In the case that said group is substituted by two or more of said substituents, these substituents may be the same or different.

Preferred examples of divalent linking groups  $L$ , to use in combination with cyan dye forming coupler moieties, include  $-\text{O}-$ ,  $-\text{NH}-$ ,  $-\text{S}-$ , substituted and

unsubstituted phenoxy, alkoxy,  $-\text{NH}-\text{SO}_2-$ , and  $-\text{N}\equiv\text{N}-$ .

Preferred examples of cyan dye forming coupler monomers comprising preferred COUP and L moieties include the following:



-continued





In formulae M-I, M-II, M-III, M-IV, M-V, M-VI, and M-VII above:

R<sub>1</sub> and R<sub>2</sub> each independently represent a conventional substituent which is well known as a substituent on the 1-position or on the 3-position of a 2-pyrazolin-5-one coupler, such as an alkyl group, a substituted alkyl group (such as a halo-alkyl group, e.g., fluoroalkyl, or cyano-alkyl, or benzyl-alkyl), an aryl group or a substituted aryl group (e.g., methyl or ethyl substituted), an alkoxy group (such as methoxy or ethoxy), an aryloxy group (such as phenoxy), an alkoxy carbonyl group (such as methoxy carbonyl), an acylamino group (such as acetyl amino), a carbamoyl group, an alkylcarbamoyl group (such as methylcarbamoyl or ethylcarbamoyl), a dialkylcarbamoyl group (such as dimethylcarbamoyl), an arylcarbamoyl group (such as phenylcarbamoyl), an alkylsulfonyl group (such as methylsulfonyl), an arylsulfonyl group (such as phenylsulfonyl), an alkylsulfonamido group (such as methanesulfonamido), an arylsulfonamido group (such as phenylsulfonamido), a sulfamoyl group, an alkylsulfamoyl group (such as ethylsulfamoyl), a dialkylsulfamoyl group (such as dimethylsulfamoyl), an arylsulfamoyl group, an alkylthio group (such as methylthio), an arylthio group (such as phenylthio), cyano group, nitro group, a halogen atom (such as fluorine atom, chlorine atom, bromine atom), etc. In case said group is substituted by two or more of said substituents, these may be the same or different. The most preferred substituents are a halogen atom, an alkyl group, an alkoxy group, an alkoxy carbonyl group, and the cyano group.

R<sub>3</sub>, R<sub>4</sub>, R<sub>5</sub>, and R<sub>6</sub> are each independently a hydrogen atom or hydroxyl group, or represent an unsubstituted or substituted alkyl group (preferably having from 1 to 20 carbon atoms, such as methyl, propyl, t-butyl, or trifluoromethyl, tridecyl), an aryl group (preferably having from 6 to 20 carbon atoms, such as phenyl, 4-t-butylphenyl, 2,4-di-t-amylphenyl, or 4-methoxyphenyl), a heterocyclic group (such as 2-furyl, 2-thienyl, 2-

pyrimidinyl, or 2-benzthiazolyl), an alkylamino group (preferably having from 1 to 20 carbon atoms, such as methylamino, diethylamino, t-butylamino), an acylamino group (preferably having from 2 to 20 carbon atoms, such as acetyl amino, propylamido, benzamido), an anilino group (such as phenylamino, 2-chloroanilino), an alkoxy carbonyl group (preferably having from 2 to 20 carbon atoms, such as methoxycarbonyl, butoxycarbonyl, 2-ethylhexyloxycarbonyl), an alkylcarbonyl group (preferably having from 2 to 20 carbon atoms, such as acetyl, butylcarbonyl, cyclohexylcarbonyl), an arylcarbonyl group (preferably having from 7 to 20 carbon atoms, such as benzoyl, or 4-t-butylbenzoyl), an alkylthio group (preferably having from 1 to 20 carbon atoms, such as methylthio, octylthio, 2-phenoxyethylthio), an arylthio group (preferably having from 6 to 20 carbon atoms, such as phenylthio, 2-butoxy-5-t-octylphenylthio), a carbamoyl group (preferably having from 1 to 20 carbon atoms, such as N-ethylcarbamoyl, N,N-dibutylcarbamoyl, N-methyl-N-butylcarbamoyl), a sulfamoyl group (preferably NH<sub>2</sub>SO<sub>2</sub> and a group having from 1 to 20 carbon atoms, such as N-ethylsulfamoyl, N,N-diethylsulfamoyl, N,N-dipropylsulfamoyl), or an alkyl sulfonamido group (preferably having from 6 to 20 carbon atoms, such as benzenesulfonamido, p-toluenesulfonamido).

Preferred examples of divalent linking groups L, to use in combination with magenta dye forming coupler moieties, include —O—, —NH—, —S—, substituted and unsubstituted phenoxy, substituted and unsubstituted aryl thiol, —NH-SO<sub>2</sub>—, substituted and unsubstituted pyrazole, substituted and unsubstituted imidazole, substituted and unsubstituted 1,2,4-triazole, and —N=N—.

Preferred examples of magenta dye forming coupler monomers comprising preferred COUP and L moieties include the following:





5,354,642

15

-continued



16

-continued

m-xvii



-continued



COUP may represent a coupler moiety, capable of forming a yellow dye by coupling with an aromatic primary amine developing agent. Couplers which form yellow dyes upon reaction with oxidized color developing agent are described in such representative U.S. Pat. Nos. as 2,298,443, 2,875,057, 2,407,210, 3,265,506, 3,384,657, 3,408,194, 3,415,652, 3,447,928, 3,542,840, 4,046,575, 3,894,875, 4,095,983, 4,182,630, 4,203,768, 4,221,860, 4,326,024, 4,401,752, 4,443,536, 4,529,691, 4,587,205, 4,587,207 and 4,617,256, and in European Patent Applications 0 259 864 A2, 0 283 938 A1, and 0 316 955 A3, the disclosures of which are incorporated by reference. Preferred yellow dye image forming couplers are acylacetamides, such as benzoylacetanilides and pivalylacetanilides, which can form heat transferable dyes upon reaction with oxidized color developing agent. Preferred coupler moieties COUP which form yellow dyes upon reaction with oxidized color developing agents are of the acylacetanilide type (formula Y-I) and benzoylacetanilide type (formulae Y-II and Y-III); the asterisk mark indicates the position of the bond to the divalent linking group L in formula (I)



Y-I



In formulae Y-I, Y-II, and Y-III above:

10 R<sub>1</sub>, R<sub>2</sub>, R<sub>3</sub>, R<sub>4</sub>, and R<sub>5</sub> each independently represents a hydrogen atom or a substituent which is conventional and well known in a yellow coupler group, for example, an alkyl group, an alkenyl group, an alkoxy group, an alkoxy carbonyl group, a halogen atom, an alkoxycarbamoyl group, an aliphatic amido group, an alkylsulfamoyl group, an alkylsulfonamido group, an alkylureido group, an alkylsubstituted succinimido group, an aryloxy group, an aryloxycarbonyl group, an arylcarbamoyl group, an arylamido group, an arylsulfamoyl group, an arylsulfonamido group, an arylureido group, carboxyl group, sulfo group, nitro group, cyano group, or thiocyanato group.

15 Preferred examples of divalent linking groups L, to use in combination with yellow dye forming coupler moieties, include —O—, —NH—, —S—, substituted and unsubstituted phenoxy, substituted and unsubstituted hydantoin, substituted and unsubstituted aryl thiol, —NH—SO<sub>2</sub>—, substituted and unsubstituted pyrazole, substituted and unsubstituted imidazole, substituted and unsubstituted 1,2,4-triazole, substituted and unsubstituted urazole, substituted and unsubstituted 1,2,3,4-tetrazole-5-one, substituted and unsubstituted benztriazole, substituted and unsubstituted benzimidazole, and substituted and unsubstituted phthalimide.

20 30 35 Preferred examples of yellow dye forming coupler monomers comprising preferred COUP and L moieties include the following:



-continued



y-iii



y-iv



y-v



y-vi



y-vii

-continued



y-viii



y-ix



y-x



y-xi



y-xii



y-xiii

-continued

y-xiv



y-xv



y-xvi



y-xvii



y-xviii



y-xix



-continued



y-xx



y-xxi



y-xxii



y-xxiii



y-xxiv

-continued



y-xxv



V- xxvi



y-xxvii



y-xxviii



V-xxix

-continued

y- xxx



y-xxxii



y-xxxii



y-xxxiii



y-xxxiv



y-xxxv



-continued



y-xxxvi



y-xxxvii



y-xxxvii



y-xxxix



y-x1



y-xli



-continued

y-xlii



y-xliii



y-xliv



y-xlv



y-xlivi

The polymeric couplers of the present invention may include homopolymers of any ethylenic monomeric couplers, copolymers of two or more ethylenic monomeric couplers, and copolymers of at least one ethylenic monomeric coupler and at least one non-color forming ethylenic monomer which does not couple with the oxidation product of a primary amine developing agent. Copolymers of ethylenic monomeric couplers and non-color forming ethylenic monomers are preferred.

Examples of non-color forming ethylenic monomers which do not couple with the oxidation product of a primary amine developing agent include acrylic acid,  $\alpha$ -chloroacrylic acid, methacrylic acid, acrylamide, methacrylamide, n-butylacrylamide, t-butylacrylamide,

diacetone acrylamide, methyl acrylate, ethyl acrylate, n-propyl acrylate, isopropyl acrylate, n-butyl acrylate, t-butyl acrylate, isobutyl acrylate, hexyl acrylate, 2-ethylhexyl acrylate, n-octyl acrylate, lauryl acrylate, 3-acroyl propanesulfonic acid, acetoacetoxyethyl acrylate, acetoxyethyl acrylate, phenyl acrylate, 2-methoxy acrylate, 2-ethoxy acrylate, 2-(2-methoxyethoxy)ethyl acrylate, methyl methacrylate, ethyl methacrylate, n-propyl methacrylate, isopropyl methacrylate, n-butyl methacrylate, t-butyl methacrylate, isobutyl methacrylate,  $\beta$ -hydroxy methacrylate, cyclohexyl methacrylate, 2-hydroxyethyl methacrylate, tetrahydrofurfuryl methacrylate, epoxyethyl methacrylate, vinyl acetate, vinyl

propionate, vinyl butyrate, vinyl laurate, vinylmethoxy acetate, vinyl benzoate, acrylonitrile, methacrylonitrile, styrene, vinyl toluene, divinyl benzene, vinyl acetophenone, sulfostyrene, triethyl styrene, isopropyl styrene, butyl styrene, chloromethyl styrene, methoxy styrene, 5 butoxy styrene acetoxy styrene, chlorostyrene, dichlorostyrene, bromostyrene, 2-methyl styrene, styrene sulfinic acid, itaconic acid, diethyl itaconate, dibutyl itaconate, citraconic acid, crotonic acid, butyl crotonate, hexyl crotonate, vinylidene chloride, vinyl methyl ether, vinyl ethyl ether, vinyl butyl ether, vinyl hexyl ether, vinyl methoxyethyl ether, vinyl dimethylaminoethyl ether, N-vinyl-2-pyrrolidone, N-vinylpyridine, 2-vinylpyridine, 4-vinylpyridine, diethyl maleate, 10 dimethyl maleate, dibutyl maleate, diethyl fumarate, dimethyl fumarate, dibutyl fumarate, acrylamide, methyl acrylamide, ethyl acrylamide, isopropyl acrylamide, n-butyl acrylamide, hydroxymethyl acrylamide, diacetone acrylamide, acryloyl morpholine, acrylamido-2-methylpropanesulfonate, methyl methacrylamide, ethyl 20 methacrylamide, n-butyl methacrylamide, t-butyl methacrylamide, 2-methoxy methacrylamide, dimethyl, diethyl methacrylamide, allyl acetate, vinyl methyl ketone, vinyl methacrylamide sulfonic acid, other acrylic acids, other  $\alpha$ -alkyl acrylates, other esters derived from 25 acrylic acids, other amides derived from acrylic acids, other vinyl esters, other aromatic vinyl compounds, other vinyl alkyl ethers, other esters of itaconic acid, other esters of fumaric acid, other esters of maleic acid, alkali and ammonium salts of sulfonic acids, alkali and 30 ammonium salts of sulfinic acids, and other vinyl ketones.

Of these non-color forming ethylenic monomers, acrylalkylsulfonates, methacryloyloxyalkylsulfonates, acrylamidoalkylsulfates, methacrylamidoalkylsulfonates, alkali and ammonium salts of these sulfonates, esters of acrylic acid, esters of methacrylic acid, and esters of maleic acid are particularly preferred. Two or more such non-color forming ethylenic monomers may be used together and in any desired combination so as to obtain desired physical and chemical properties such as solubility, gelatin compatibility, flexibility, and thermal stability in the resulting polymer. For example, the combinations of methyl acrylate and butyl acrylate, 40 butyl acrylate and styrene, butyl methacrylate and methacrylic acid, methyl acrylate and diacetone acrylamide, potassium styrenesulfinate and sodium acrylamido-2-methylpropanesulfonate, acetoacetoxyethyl methacrylate and sodium 3-acryloylpropanesulfonate, potassium styrenesulfinate and sodium acryloyloxypropane sulfonate can be used.

It will be understood by one skilled in the art that the above listed coupler moieties, non-color forming monomeric moieties, linking groups, and polymeric backbone groups are representative and not exclusive. Further examples of such groups usable in the present invention are disclosed in U. Pat. Nos. 4,584,267 and 4,948,698, the disclosures of which are incorporated by reference above.

Polymeric couplers of the present invention may be 60 prepared by any radical polymerization method well known in the art. Polymeric couplers of the present invention may be prepared by emulsion polymerization as is described in *Emulsion Polymerization* (F. A. Bovey, Interscience Publishers, New York, 1955), in U.S. application Ser. Nos. 387,128 and 377,271, in European Patent Application Nos. 0 259 864 A2 and 0 316 955 A3, and in U.S. Pat. Nos. 4,367,282, 4,388,404, 4,435,503,

4,436,808, 4,444,870, and 4,522,916, the disclosures of which are incorporated herein by reference.

Polymeric couplers of the present invention may be prepared by solution polymerization methods as described in U. Pat. Nos. 4,455,368, 4,474,870, 4,436,808, 4,455,366, 4,522,916, 4,540,654, 4,576,910, 4,668,613, European Patent No. 0 259 864 B1, European Patent Application No. 0 283 938 A1, and in U.S. application Ser. No. 7/879,044, filed May 6, 1992 by Chen et al., the disclosures of which are incorporated herein by reference.

Polymeric couplers of the present invention may be prepared by radical polymerization methods using chain transfer agents to produce a class of polymeric couplers known as telomeric couplers. Such methods are described in U.S. Pat. No. 4,874,689 and in European Patent Application No. 0 3 16 955 A3, the disclosures of which are incorporated herein by reference.

Polymeric couplers of the present invention may be prepared by radical polymerization methods using microemulsion polymerization techniques as described in U.S. application Ser. No. 7/796,107, filed Nov. 21, 1991 by Texter et al., now U.S. Pat. No. 5,234,807 the disclosure of which is incorporated herein in its entirety.

It is preferred that the molecular weight of the polymeric couplers of the present invention be in the range of 5,000 to 10,000,000. It is more preferred that the molecular weight of the polymeric couplers of the present invention be in the range of 10,000 to 2,000,000. It is undesirable for the molecular weight of the polymeric couplers of the present invention to be too low, because unwanted thermal diffusion transfer of said couplers might then occur. It is preferred that the molecular weight of the polymeric couplers of the present invention not be so large as to make their coating difficult or so large as to make their dispersal in a form suitable for coating in a photographic colloid difficult.

Exposed photographic elements containing coupler compounds of formula (I) according to the invention are developed with a color developer solution in order to form a heat transferable dye image. In principle, any combination of developer agent and polymeric coupler compound which forms a heat transferable dye upon development may be used. Selection of substituents for the polymeric coupler compounds of the invention as well as the developer agent will affect whether a heat transferable dye is formed upon development. Whether a particular coupler compound and developer agent combination generates a heat transferable dye suitable for use in the present invention will be readily ascertainable to one skilled in the art through routine experimentation.

Preferred color developing agents useful in the invention are p-phenylenediamines. Especially preferred are: 4-amino-N,N-diethylaniline hydrochloride; 4-amino-3-methyl-N,N-diethylaniline hydrochloride; 4-amino-3-methyl-N-ethyl-N-(p-methanesulfonylamidoethyl)aniline sulfate hydrate; 4-amino-3-methyl-N-ethyl-N-(p-hydroxyethyl)aniline sulfate; 4-amino-3-(p-methanesulfonamido)ethyl-N,N-diethylaniline hydrochloride; 4-amino-3-methyl-N-ethyl-N-(p-methanesulfonamidoethyl)aniline sesquisulfate monohydrate; and 4-amino-3-methyl-N-ethyl-N-(2-methoxyethyl)aniline di-p-toluenesulfonic acid.

Photographic elements in which the photographic couplers of formula (I) are incorporated can be simple elements comprising a support and a single silver halide emulsion layer, or they can be multilayer, multicolor elements. The silver halide emulsion layer can contain, or have associated therewith, other photographic addenda conventionally contained in such layers.

A typical multilayer, multicolor photographic element according to this invention comprises a support having thereon a red sensitive silver halide emulsion layer having associated therewith a cyan dye image forming coupler compound, a green-sensitive silver halide emulsion layer having associated therewith a magenta dye image forming coupler compound and a blue sensitive silver halide emulsion layer having associated therewith a yellow dye image forming coupler compound. Each silver halide emulsion layer can be composed of one or more layers and the layers can be arranged in different locations with respect to one another. Typical arrangements are described in *Research Disclosure*, Issue Number 308, pp. 993-1015, published December, 1989 (hereafter referred to as "Research Disclosure"), the disclosure of which is incorporated by reference.

The light sensitive silver halide emulsions can include coarse, regular or fine grain silver halide crystals of any shape or mixtures thereof and can be comprised of such silver halides as silver chloride, silver bromide, silver bromoiodide, silver chlorobromide, silver chloroiodide, silver chlorobromoiodide and mixtures thereof. The emulsions can be negative working or direct positive emulsions. They can form latent images predominantly on the surface of the silver halide grains or predominantly on the interior of the silver halide grains. They can be chemically or spectrally sensitized. The emulsions typically will be gelatin emulsions although other hydrophilic colloids as disclosed in *Research Disclosure* can be used in accordance with usual practice.

The support can be of any suitable material used with photographic elements. Typically, a flexible support is employed, such as a polymeric film or paper support. Such supports include cellulose nitrate, cellulose acetate, polyvinyl acetal, poly(ethylene terephthalate), polycarbonate, white polyester (polyester with white pigment incorporated therein) and other resinous materials as well as glass, paper or metal. Paper supports can be acetylated or coated with baryta and/or an alpha-olefin polymer, particularly a polymer of an alpha-olefin containing 2 to 10 carbon atoms such as polyethylene, polypropylene or ethylene butene copolymers. The support may be any desired thickness, depending upon the desired end use of the element. In general, polymeric supports are usually from about 3  $\mu\text{m}$  to about 200  $\mu\text{m}$  and paper supports are generally from about 50  $\mu\text{m}$  to about 1000  $\mu\text{m}$ .

The dye receiving layer to which the formed dye image is transferred according to the process of the invention may be present as a coated or laminated layer between the support and silver halide emulsion layer(s) of the photographic element, or the photographic element support itself may function as the dye receiving layer. Alternatively, the dye receiving layer may be in a separate dye receiving element which is brought into contact with the photographic element before or during the dye transfer step. If present in a separate receiving element, the dye receiving layer may be coated or laminated to a support such as those described for the photographic element support above, or may be self-support-

ing. In a preferred embodiment of the invention, the dye-receiving layer is present between the support and silver halide emulsion layer of an integral photographic element.

5 The dye receiving layer may comprise any material effective at receiving the heat transferable dye image. Examples of suitable receiver materials include polycarbonates, polyurethanes, polyesters, polyvinyl chlorides, poly(styrene-coacrylonitrile)s, poly(caprolactone)s and mixtures thereof. The dye receiving layer may be present in any amount which is effective for the intended purpose. In general, good results have been obtained at a concentration of from about 1 to about 10 g/m<sup>2</sup> when coated on a support. In a preferred embodiment of the invention, the dye receiving layer comprises a polycarbonate. The term polycarbonate as used herein means a polyester of carbonic acid and a glycol or a dihydric phenol. Examples of such glycols or dihydric phenols are paraxylene glycol, 2,2-bis(4-oxyphenyl) propane, bis(4-oxyphenyl)methane, 1,1-bis(4-oxyphenyl) ethane, 1,1-bis(oxyphenyl)butane, 1,1-bis(oxyphenyl) cyclohexane, 2,2-bis(oxyphenyl)butane, etc. In a particularly preferred embodiment, a bisphenol-A polycarbonate having a number average molecular weight of at least 15 about 25,000 is used. Examples of preferred polycarbonates include General Electric LEXAN® Polycarbonate Resin and Bayer AG MACROLON 5700®. Further, a thermal dye transfer overcoat polymer as described in U. Pat. No. 4,775,657 may also be used. Heating times of from about 10 seconds to 30 minutes at temperatures of from about 50° to 200° C. (more preferably 75° to 160° C., and most preferably 80° to 120° C.) are preferably used to activate the thermal transfer process. This aspect makes it possible to use receiver polymers that have a relatively high glass transition temperature (T<sub>g</sub>) (e.g., greater than 100° C.) and still effect good transfer, while minimizing back transfer of dye (diffusion of dye out of the receiver onto or into a contact material).

20 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935

Automated stripping techniques applicable to the present invention are disclosed in copending U.S. application Ser. No. 7/805,717, filed Dec. 6, 1991, of Texter et al., now U.S. Pat. No. 5,164,280 the disclosure of which is incorporated by reference.

Further details regarding silver halide emulsions and elements, and addenda incorporated therein can be found in Research Disclosure, referred to above.

The terms "in association" or "associated with" are intended to mean that materials can be in either the same or different layers, so long as the materials are accessible to one another.

Photographic elements as described above are exposed in the process of the invention. Exposure is generally to actinic radiation, typically in the visible region of the spectrum, to form a latent image as described in Research Disclosure Section XVIII. The exposure step may also include exposure to radiation outside the visible region. The following examples are provided to help further illustrate the invention.

### EXAMPLES 1-2

#### Preparation of Yellow Monomer (Y1)

The structure of Y1 is identical to that of y-i illustrated earlier in the specification. In a 5L 3-neck round-bottomed flask, equipped with an addition funnel, mechanical stirrer, and thermometer, about 600 g (2.1 mol) of starting material i was dissolved in 3 L of toluene while stirring under nitrogen; a yellow solution resulted. About 190 mL (2.3 mol) of sulfonyl chloride was added dropwise over a 45 minute period while maintaining the temperature below 25° C. After about 3 hours, thin layer chromatography (TLC) indicated a trace of starting material was still present; an additional 10 mL of sulfonyl chloride was then added to drive the reaction to completion. The toluene was then removed by rotary evaporation and the brown oil obtained was mixed with about 500 mL of hexanes, and a white crystalline product, intermediate ii, was obtained.



5 The volume of ice/HCl (50:50 by weight). The organic layer was washed three times with about 100 mL of 10% aqueous HCl, and the yellow aqueous layer was washed three times with about 100 mL of ethyl acetate. The 10 organic fraction was concentrated to give a yellow solid; this fraction was triturated with about 250 mL of methanol to give a white crystalline solid. This solid was washed with methanol and yielded about 208 g of intermediate iii. The filtrate was concentrated and washed twice with 50 mL of water, and yielded an additional 15.9 g of iii. The nitro group in iii was reduced to the primary amine to yield intermediate iv by catalytic (Raney cobalt; RaCo) reduction. About 614 g (1.44 mol) of iii was dissolved in about 7L tetrahydrofuran (THF) and combined with about 150 g of prereduced RaCo; hydrogen pressure was maintained at about 450 psi for 3 hours at about 28° C. to effect complete reaction.

20 About 15.2 g (38.5 mmol) of iv in about 50 mL of THF was stirred in a 250 mL 3-neck round-bottomed flask equipped with a thermometer and addition funnel.



In a 2-L 3-neck round-bottomed flask equipped with a mechanical stirrer and thermometer, about 95 g (0.68 mol) of p-nitrophenol and about 200 g (0.62 mol) of intermediate ii were dissolved in about 800 mL of dimethylformamide (DMF) to produce an orange-brown solution. This solution was heated to 40° C., and tetramethylquandine (TMG; about 143 g, 1.2 mol) was then added dropwise over a period of 30 minutes. During this period the reaction mixture darkened, turned red, and the temperature rose to about 60° C. Thereafter, the reaction mixture was maintained at about 50° C. for about 3.5 hours, during which time the reaction went to completion. After cooling the mixture to room temperature, about 1 L of ethyl acetate was added and then the mixture was quenched by adding to a 1 L

55 The light brown solution was cooled to about 5° C. About 3.5 mL (42.2 mmol) of acryloyl chloride was added dropwise over a period of about 15 minutes while keeping the reaction temperature below 15° C. The 60 brown solution was poured slowly into a rapidly stirring mixture of 20 mL HCl (concentrated), 200 mL ice, and 20 mL water. A brown precipitate formed immediately. This precipitate was filtered, washed with water, and sucked dry overnight. The product was then placed in a 40° C. vacuum oven and dried to yield 16.5 g of Y1.

## Preparation of Polymeric Coupler Y2



Deionized water (about 100 g), about 2.08 g of 20% (w/w) sodium N-methyl-N-oleoyltaurate (Igepon T-77), and about 10 g of acetone were mixed in a 250 mL 4-necked roundbottom flask equipped with a mechanical stirrer, nitrogen inlet, and condenser. The flask was immersed in a constant temperature bath at 80° C. and heated for 30 min with nitrogen purging. A monomer solution comprising about 4.493 g of monomer Y1 (0.01 mol), about 3.846 g of butyl acrylate (0.03 mol), and about 50 mL of N,N-dimethylformamide was prepared. About 2 g of 5% (w/w) ammonium persulfate was added to the reactor and stirred for 3 min. The monomer solution was then pumped into the reactor over 2.5 h. The polymerization was continued for 8 h. The latex suspension was then cooled, filtered, and dialyzed against distilled water overnight. The latex was then concentrated to about 7.8% (w/w) solids with an Amicon ultrafiltration unit. The z-average particle size measured by a Malvern Autosizer IIC was about 95 nm. The elemental analysis results were: C (60.76%); H (6.93%); N (3.47%); Cl (4.97%).

## Preparation of Comparison Coupler (Y3) Dispersion



About 8 g of Y3 were dissolved in about 24 g of ethyl acetate at about 60° C. An aqueous gelatin solution comprising about 3.2 g of 10% (w/w) Alkanol-XC (Du Pont), about 19.2 g 12.5% (w/w) aqueous gelatin, and about 19.2 g water was prepared. These aqueous and ethyl acetate solutions were then combined with stirring and passed through a colloid mill five times to obtain a fine particle dispersion of Y3. The resulting dispersion was chill set, noodled, and washed for about 4 h to remove the ethyl acetate. This dispersion was then remelted, chill set, and stored until use.

## Preparation of Thermal Solvent Dispersion

An aqueous solution was prepared at about 50° C. by combining about 3.75 g of 10% (w/w) aqueous Alkanol XC (Du Pont), about 30 g of 12.5% (w/w) gelatin, and about 78.75 g water. About 12.5 g of p-hydroxy-2-ethyl-

(Y2) hexyl benzoate (Pfaltz and Bauer) was added to this solution with stirring, and this coarse emulsion was then passed through a colloid mill five times to produce a fine particle sized dispersion. This dispersion was then 5 chill set and stored in the cold until used.

## Coating Support and Receiver

A reflection base paper material, resin coated with high density polyethylene, was coated with a mixture of 10 polycarbonate, polycaprolactone, and 1,4-didecyloxy-2,5-dimethoxy benzene at a 0.77:0.115:0.115 weight ratio respectively, at a total coverage of 3.28 g/m<sup>2</sup>.

## Preparation of Test Coatings

15 The test coating structure comprised two layers coated on the receiver support described above. The receiver support was subjected to corona discharge bombardment within about 24 h prior to coating the test elements. The first layer contained gelatin at a coverage of about 1.07 g/m<sup>2</sup>, thermal solvent (p-hydroxy-2-ethylhexyl benzoate) at a coverage of about 1.07 g/m<sup>2</sup>, and blue sensitized silver chloride at a coverage of about 540 mg/m<sup>2</sup> as silver. In the control coating 1, the dispersion of Y3 was coated to yield a Y3 coverage of about 1.07 g/m<sup>2</sup>. The coating 2 of polymeric coupler Y2 contained a molar equivalent of coupling sites and a corresponding coverage of about 1.38 g/m<sup>2</sup>. This first layer was overcoated with a second layer. The second layer contained gelatin at a coverage of about 1.07 g/m<sup>2</sup>. Hardener, 1,1'-[methylene bis(sulfonyl)]bis-ethene (MBSE), was coated at a coverage of about 32.1 mg/m<sup>2</sup> to crosslink the gelatin.

## Evaluation

35 These test coatings were exposed and processed for 45" at 95° F. in a developer solution comprising the following:

|         |                                                                |         |
|---------|----------------------------------------------------------------|---------|
| (Y3) 40 | Triethanolamine                                                | 12.41 g |
|         | Phorwite REU (Mobay)                                           | 2.3 g   |
|         | Lithium polystyrene sulfonate<br>(30% aqueous solution)        | 0.30 g  |
|         | N,N-diethylhydroxylamine<br>(85% aqueous solution)             | 5.40 g  |
| 45      | Lithium sulfate                                                | 2.70 g  |
|         | KODAK Color Developing Agent CD-3                              | 5.00 g  |
|         | 1-Hydroxyethyl-1,1-diphosphonic acid<br>(60% aqueous solution) | 1.16 g  |
|         | Potassium carbonate, anhydrous                                 | 21.16 g |
| 50      | Potassium chloride                                             | 1.60 g  |
|         | Potassium bromide                                              | 7.0 mg  |
|         | Water to make one liter                                        |         |
|         | pH = 10.04 @ 27° C.                                            |         |

These coatings were then dipped in a stop bath (10% (w/w) acetic acid; 60"), rinsed (60" in pH 7 phthalate buffer (VWR); 5 min in water rinse), and dried. The test coatings were then passed through pinch rollers heated to 110° C. under a nip pressure of 20 psi at a rate of 0.25 ips (inches per second). The test coatings were passed through with the emulsion/dye forming and gelatin overcoat layers in contact with the gelatin coated side of a stripping adhesion sheet, as described in U.S. application Ser. No. 7/805,717, now U.S. Pat. No. 5,164,280. This adhesion sheet was subsequently removed by shear from the test element, thereby removing the emulsion/dye forming and gelatin overcoat layers from the receiver/base support. The resulting transferred dye scale was read by reflection densitometry and/or by reflec-

tance spectroscopy. The receiver and donor (spent dye forming layer) elements were examined imagewise by extracting residual coupler and dye, as determined by HPLC (high performance liquid chromatography).

These coatings were processed as described above, whereby the test coatings were passed through the aforesaid pinch rollers once, and the resulting reflection densitometry (status A filters) is illustrated in FIG. 1. This densitometry shows that the coating of the present invention, Example 2, comprising polymeric coupler Y2, is considerably more active (curve 2) than the coating of the comparison Example 1 (curve 1), comprising coupler Y3. A benefit that can be derived from using polymeric couplers of enhanced reactivity, is that the same amount of dye density can be obtained, as obtained with a conventional coupler dispersion of lower activity, with less coated silver halide and/or with less coated coupler (on an equivalent basis).

Several additional sets of these coatings were processed as described above, except that they were passed through the aforesaid pinch rollers ten times before stripping the donor layers from the receiver/base element. Regions of these strips were then read by reflectance spectroscopy to obtain visible spectra of the transferred dye. These spectra are illustrated in FIG. 2.

TABLE 1

| Coupler Y3 and Dye Distribution            |        |                |                                    |                             |
|--------------------------------------------|--------|----------------|------------------------------------|-----------------------------|
| Coating                                    | Region | Donor/Receiver | Coupler Y3<br>(mg/m <sup>2</sup> ) | Dye<br>(mg/m <sup>2</sup> ) |
| Example 1<br>(Comparison)                  | Dmin   | Donor          | 433                                | 0                           |
|                                            |        | Receiver       | 551                                | 0                           |
| Example 2<br>(Present<br>Invention;<br>Y2) | Dmax   | Donor          | 350                                | 48                          |
|                                            |        | Receiver       | 466                                | 87                          |

Curve 1 in FIG. 2 corresponds to the comparison coating of Example 1, which comprises the conventional coupler Y3. This curve was obtained at a reflectance density Dmax of 0.24. Curve 2 in FIG. 2 corresponds to the coating of the present invention, Example 2, comprising polymeric coupler Y2. This curve was obtained at a reflectance density Dmax of 0.45. The long wavelength absorption evident in curve 1 provides a brownish discoloration to the hue obtained, relative to that obtained in curve 2 for the polymeric coupler generated dye of the present invention. Some of these additional sets of processed coatings, including both the separated donor and receiver elements, were analyzed by extracting punches taken from Dmax and Dmin regions. These extracts were analyzed by HPLC to determine the amount of coupler and dye present; the results are shown in Table 1. The same dye is generated by coupler Y3 and by polymeric coupler Y2. In the comparison Example 1, 135 mg/m<sup>2</sup> of dye remained in the donor and receiver layers after thermal dye transfer processing, and in the Example 2 of the present invention, 441 mg/m<sup>2</sup> of dye remained in the donor and receiver elements after dye transfer. These extraction results corroborate the Dmax densitometry illustrated in FIG. 1, and show that the polymeric coupler Y2 is significantly more active than the conventionally dispersed coupler Y3. Table 1 also dramatically illustrates the distribution of coupler Y3 and dye among the donor and receiver layers after thermal transfer. In the Dmin region of Example 1, more coupler Y3 ends up in the receiver layer than in the donor. In the Dmax region of Example

1, a comparable amount of coupler Y3 is transferred to the receiver. In Example 2, however, there is no monomeric coupler to be transferred to the receiver, since dye is formed by reaction of oxidized developer with polymeric coupler Y2.

## EXAMPLES 3-4



About 5 g of Y1, about 4.5 g of butyl acrylate, about 0.5 g of N-acrylamido-2,2'-dimethylpropane sulfonic acid (sodium salt), and about 40 mL of N,N-dimethylformamide were mixed in a 3-neck 100-mL roundbottom flask. The flask was immersed in a constant temperature bath at 80° C. and purged with nitrogen for 30 min. About 0.25 g of 2,2'-azobis(2-methylpropionitrile) was then added, and the polymerization was continued for about 4 h. The polymer solution was then diluted with about 120 mL of methanol and then dispersed into about 300 mL of hot water (about 70° C.) with vigorous stirring. The resulting latex was then concentrated to 3.63% solids with an Amicon ultrafiltration unit. The z-average particle size measured with a Malvern Autosizer IIC was 59 nm. The elemental analysis results were: C (60.1%); H (6.79%); N (3.66%).

## Preparation of Test Coatings

A test coating structure and format identical to that described above for Examples 1 and 2 was utilized, except that lower levels of coupler Y3 (859 mg/m<sup>2</sup>; Example 3) and polymeric coupler Y4 (1.11 g/m<sup>2</sup>; a molar equivalent of coupling sites relative to the coated level of Y3, Example 4) were coated. The same coating support and receiver were utilized.

TABLE 2

| Coupler Y3 and Yellow Dye Transferred to Receiver |        |                                    |                             |
|---------------------------------------------------|--------|------------------------------------|-----------------------------|
| Coating                                           | Region | Coupler Y3<br>(mg/m <sup>2</sup> ) | Dye<br>(mg/m <sup>2</sup> ) |
| Example 3<br>(Comparison)                         | Dmin   | 419                                | 29                          |
|                                                   | Dmax   | 268                                | 143                         |
| Example 4<br>(Present Invention;<br>Y4)           | Dmin   | 0                                  | 10                          |
|                                                   | Dmax   | 0                                  | 178                         |

An identically prepared thermal solvent dispersion of p-hydroxy-2-ethylhexyl benzoate was used, and this thermal solvent was coated at the same level of 1.07 g/m<sup>2</sup>. This same level of gelatin was coated in the first and second (overcoat) layers, and the same hardener, MBSE, was coated identically, as described earlier, to crosslink the gelatin.

## Evaluation

Several sets of these coatings were exposed and processed as described above for Examples 1 and 2; the same wet development solution, stop bath, buffer bath, and wash sequence was used. Thermal transfer was then activated by passing these test coatings through the heated pinch rollers at 110° C. ten times as earlier described. The silver halide and dye forming layer and overcoat were removed using the adhesion sheet stripping method described above. The receiver elements were then examined by status A densitometry (FIG. 3) and by HPLC extraction analysis for transferred coupler Y3 and transferred dye. The densitometry illustrated in FIG. 3 shows that the polymeric coupler Y4 yields a higher Dmax than does the conventional dispersion of the coupler Y3. Both Y3 and Y4 produce the same dye on reaction with the oxidized developer.

HPLC analysis of the Drain and Dmax regions of these coatings for transferred coupler Y3 and for transferred dye is illustrated in Table 2. The comparison coating of Y3 (Example 3) yielded substantial coupler transferred in both the Dmin and Dmax regions. This transfer of coupler was not observed in the coating of the present invention (Example 4), due to the immobility of the polymeric coupler Y4 and the lack of Y3 in the test coating. Dye was transferred in both of these coatings. The coating of this invention (Example 4) yielded a higher level of transferred dye in the Dmax region and a lower level in the Drain region.

## EXAMPLES 5-6

## Preparation of Cyan Monomer (C1)

The structure of monomer C1 is identical to that of monomer c-i shown earlier in the specification. About 34.8 g (0.16 mol) of 1,4-dihydroxy-N-methyl-2-naphthalenecarboxamide, about 25 g (0.16 mol) of 2-fluoro-5-nitroaniline, and about 100 mL of dry dimethylfornamide (DMF) were placed in a 500-mL three-necked flask set in an ice bath. The mixture was cooled under nitrogen to about 0° to 5° C. About 9.6 g (0.32 mol) of sodium hydride (as an 80% by weight dispersion in mineral oil) was slowly added in portions over the course of about an hour, with intervals between additions to allow foaming to subside. The mixture was stirred overnight at room temperature, during which time the reaction went to completion. The mixture was drowned in about 600 mL of dilute HCl ice water. The solid was collected and washed with water, and dried in a vacuum oven at 55° C. to yield 55 g of the crude product. This crude was recrystallized form a 20:1 mixture of acetonitrile and tetrahydrofuran (THF) to yield about 32 g of intermediate v.



About 20 g (0.0566 mol) of intermediate v, about 7.0 g (0.0577 mol) of N,N-dimethylaniline, and about 150 mL of dry THF were added to a 500-mL three-necked flask set in an ice bath. The mixture was cooled under nitrogen to about 0° C. and about 5.2 g (0.0577 mol) of acryloyl chloride in about 10 mL of dry THF was slowly added from a dropping funnel, while keeping the temperature below about 5° C. The addition took about 15 to 20 minutes. The reaction mixture was stirred cold for about 2 hours, while the reaction went to completion. The reaction mixture was drowned into about a liter of ice water (to which about 2 to 3 mL of concentrated HCl was added prior to drowning). The solid was stirred for about 15 minutes, and then collected and washed with water. The product was dried overnight at 55° C., and then recrystallized twice from 20 parts by weight acetonitrile with a small amount of THF to yield 18 g of monomer C1.

Preparation of Polymeric Cyan Coupler (C2)

About 200 g deionized water, about 2.64 g of 20% (w/w) sodium N-methyl-N-oleoyltaurate (Igepon T-77), and about 20 g of acetone were mixed in a 500 mL 4-neck roundbottom flask equipped with a mechanical stirrer, nitrogen inlet, and condenser. The flask was immersed in a constant temperature bath at 80° C. and heated for 30 min with nitrogen purging. A monomer solution comprising about 4.074 g (0.01 mol) of C1, about 3.846 g of butyl acrylate (0.03 mol), and about 100 mL of N,N-dimethylformamide was prepared. About 3.16 g of 5% (w/w) aqueous ammonium persulfate was added to the reactor and stirred for 3 min. The monomer solution was then pumped into the reactor over 22 h, and the polymerization was continued for one hour. The resulting latexsuspension of C2 was cooled, filtered, and dialyzed against distilled water overnight. The latex was then concentrated to 2.53% solids with an Amicon ultrafiltration unit. The z-average particle size measured with a Malvern Autosizer IIC was about 49 nm. The elemental analysis results were: C (60.88%); H (7.28%); N (6.21%).

Preparation of Comparison Coupler (C3) Dispersion

(C3)

About 8 g of C3 were dissolved in about 24 g of ethyl acetate at about 60° C. An aqueous gelatin solution comprising about 3.2 g of 10% (w/w) Alkanol-XC, about 19.2 g 12.5% (w/w) aqueous gelatin, and about 19.2 g water was prepared. These aqueous and ethyl acetate solutions were then combined with stirring and passed through a colloid mill five times to obtain a fine particle dispersion of C3. The resulting dispersion was chill set, noodled, and washed for about 4 h to remove the ethyl acetate. This dispersion was then remelted, chill set, and stored until use.

Preparation of Test Coatings

A test coating structure and format identical to that described above for Examples 1 and 2 was utilized, except that lower levels of coupler C3 (537 mg/m<sup>2</sup>; Example 5) and polymeric coupler C2 (579 mg/m<sup>2</sup>; a molar equivalent of coupling sites relative to the coated level of C3, Example 5) were coated. The same coating support and receiver were utilized. An identically prepared thermal solvent dispersion of p-hydroxy-2-ethylhexyl benzoate was used, and this thermal solvent was coated at the same level of 1.07 g/m<sup>2</sup>. This same level of gelatin was coated in the first and second (overcoat) layers, and the same hardener, MBSE, was coated identically, as described earlier, to crosslink the gelatin.

Evaluation

Several sets of these coatings were exposed and processed as described above for Examples 1 and 2; the same wet development solution, stop bath, buffer bath, and wash sequence was used. Thermal transfer was then activated by passing these test coatings through the heated pinch rollers at 110° C. ten times as earlier described. The silver halide and dye forming layer and overcoat were removed using the adhesion sheet stripping method described above. The receiver elements were then examined by status A densitometry (FIG. 4), reflectance spectroscopy (FIG. 5), and by HPLC extraction analysis for transferred coupler C3 and transferred dye. The densitometry illustrated in FIG. 4 shows that the polymeric coupler C2 yields a lower Dmax than does the conventional dispersion of the coupler C3. Both C2 and C3 produce the same cyan dye on reaction with the oxidized developer. Note in FIG. 5, however, that the dye transferred in the comparison coating of Example 5 has a distinctly hypsochromically shifted short wavelength absorption edge. This shift yields a hue that is much more blue than is the cyan hue of the dye transferred in Example 6, from the polymeric coupler C2 of the present invention.

HPLC analysis of the Dmin and Dmax regions of these coatings for transferred coupler C3 and for trans-

ferred dye is illustrated in Table 3. The comparison coating of C3 (Example 5) yielded substantial coupler transferred in both the Dmin and Dmax regions. This transfer of coupler was not observed in the coating of the present invention (Example 6), due to the immobility of the polymeric coupler C2 and the lack of C3 in the test coating. Dye was transferred in both of these coatings. The coating of this invention (Example 6) yielded a higher level of transferred dye in the Dmax region. The apparently higher Dmax observed in the comparison coating of Example 5, illustrated as curve I in FIG. 4, may be attributed to the effectively wider absorption band and the bandwidth of the filters used in status A densitometry. The significant difference in hue illustrated in curves 1 and 2 in FIG. 5 may be attributed to the effects of the coupler (C3) transferred to the receiver in Example 5.

TABLE 3

| Coupler C3 and Cyan Dye Transferred to Receiver |        |                                 |                          |
|-------------------------------------------------|--------|---------------------------------|--------------------------|
| Coating                                         | Region | Coupler C3 (mg/m <sup>2</sup> ) | Dye (mg/m <sup>2</sup> ) |
| Example 5<br>(Comparison; C3)                   | Dmin   | 166                             | 0.6                      |
|                                                 | Dmax   | 56                              | 163                      |
| Example 6<br>(Present Invention;<br>C2)         | Dmin   | 0                               | 2.3                      |
|                                                 | Dmax   | 0                               | 196                      |

## EXAMPLES 7-9

Preparation of Polymeric Cyan Coupler (C4)

(C4)

About 300 g deionized water, about 3.96 g of 20% (w/w) sodium N-methyl-N-oleoyltaurate (Igepon T-77), and about 20 g of acetone were mixed in a 500 mL 4-neck roundbottom flask equipped with a mechanical stirrer, nitrogen inlet, and condenser. The flask was immersed in a constant temperature bath at 80° C. and heated for 30 min with nitrogen purging. A monomer solution comprising about 6.22 g (0.015 mol) of C1, about 6.487 g of ethoxyethyl acrylate (0.045 mol), and about 150 mL of N,N-dimethylformamide was prepared. About 3.16 g of 5% (w/w) aqueous ammonium persulfate was added to the reactor and stirred for 3 min. The monomer solution was then pumped into the reactor over 7 h, and the polymerization was continued for one hour. The resulting latex was cooled, filtered, and dialyzed against distilled water overnight. The latex was then concentrated to 4.33% solids with an Amicon ultrafiltration unit. The z-average particle size measured with a Malvern Autosizer IIC was about 81 nm. The elemental analysis results were: C (60.06%); H (6.6%); N (6.43%).



About 250 g deionized water, about 6 g of 20% (w/w) sodium N-methyl-N-oleoyltaurate (Igepon T-77), and about 20 g of acetone were mixed in a 500 mL 4-neck roundbottom flask equipped with a mechanical stirrer, nitrogen inlet, and condenser. The flask was immersed in a constant temperature bath at 80° C. and heated for 30 min with nitrogen purging. A monomer solution comprising about 6.11 g (0.015 mol) of C1, about 1.92 g of butyl acrylate (0.015 mol), about 3.83 g (0.015 mol) N-acrylamidoundecanoic acid, and about 150 mL of N,N-dimethylformamide was prepared. About 4.7 g of 5% (w/w) aqueous ammonium persulfate was added to the reactor and stirred for 3 min. The monomer solution was then pumped into the reactor over 7 h, and the polymerization was continued for one hour. A solution comprising about 3 g of 20% (w/w) sodium N-methyl-N-oleoyltaurate, about 2.4 g of 5% ammonium persulfate, and about 50 mL of deionized water was then added over 6 h, and the reaction was allowed to continue for an additional hour. The resulting latex was cooled, filtered, and dialyzed against distilled water overnight. The latex was then concentrated to 5.06% solids with an Amicon ultrafiltration unit. The z-average particle size measured with a Malvern Autosizer IIC was about 49 nm. The elemental analysis results were: C (62.89%); H (7.95%); N (6.45%).

#### Preparation of Test Coatings

A test coating structure and format identical to that described above for Examples 5 and 6 was utilized; and polymeric couplers C4 (562 mg/m<sup>2</sup>; Example 8) and C5 (738 mg/m<sup>2</sup>; Example 9) were coated at a molar equivalent of coupling sites, relative to the coated level of C3 (537 mg/m<sup>2</sup>) in Example 7. The same coating support and receiver were utilized. An identically prepared thermal solvent dispersion of p-hydroxy-2-ethylhexyl benzoate was used, and this thermal solvent was coated at the same level of 1.07 g/m<sup>2</sup>. This same level of gelatin was coated in the first and second (overcoat) layers, and the same hardener, MBSE, was coated identically, as described earlier, to crosslink the gelatin.

#### Evaluation

Several sets of these coatings were exposed and processed as described above for Examples 5 and 6; the same wet development solution, stop bath, buffer bath, and wash sequence were used. Thermal transfer was then activated by passing these test coatings through the heated pinch rollers at 110° C. ten times as earlier described. The silver halide and dye forming layer and overcoat were removed using the adhesion sheet stripping method described above. HPLC analysis of the Dmin and Dmax regions of the donor and receiver

elements from these coatings for transferred coupler C3 and for transferred dye is illustrated in Table 4. The comparison coating of C3 (Example 7) yielded substantial coupler transferred in both the Dmin and Dmax regions. This transfer of coupler was not observed in the coatings of the present invention (Examples 8 and 9), due to the immobility of the polymeric couplers C4 and C5 and the lack of C3 in these test coatings.

TABLE 4

| Coating                              | Region | Coupler C3 and Cyan Dye Distribution |                                 |                          |
|--------------------------------------|--------|--------------------------------------|---------------------------------|--------------------------|
|                                      |        | Donor/Receiver                       | Coupler C3 (mg/m <sup>2</sup> ) | Dye (mg/m <sup>2</sup> ) |
| Example 7<br>(Comparison; C3)        | Dmin   | Donor                                | 255                             | <1.1                     |
|                                      |        | Receiver                             | 257                             | <1.1                     |
|                                      | Dmax   | Donor                                | 49                              | 171                      |
|                                      |        | Receiver                             | 24                              | 183                      |
| Example 8<br>(Present Invention; C4) | Dmin   | Donor                                | 0                               | <1.1                     |
|                                      |        | Receiver                             | 0                               | 0.46                     |
|                                      | Dmax   | Donor                                | 0                               | 74                       |
|                                      |        | Receiver                             | 0                               | 211                      |
| Example 9<br>(Present Invention; C5) | Dmin   | Donor                                | 0                               | 2.9                      |
|                                      |        | Receiver                             | 0                               | 4.6                      |
|                                      | Dmax   | Donor                                | 0                               | 66                       |
|                                      |        | Receiver                             | 0                               | 161                      |

## EXAMPLES 10-11

## Preparation of Magenta Monomer (M1)

The structure of monomer M1 is identical to that of monomer m-ii shown earlier in the specification. To a solution of coupler vi (about 20 g, 51.4 mmol) and the disulfide vii (about 12.5 g, 28.4 mmol) in about 100 mL of DMF at room temperature was added a solution of bromine (1.45 mL, 28.3 mmol) in DMF (10 mL). This combined solution was warmed to 65° C. and stirred for 12 h, and then allowed to cool to room temperature. The mixture was slowly poured into 1L of ice water and the white precipitate was collected by suction filtration and dried to give about 35.2 g of intermediate viii.



-continued



To a slurry of viii (30.3 g, 50 mmol) in 250 methanol was added KOH (28.0 g, 500 mmol) in water (25 mL). This mixture was refluxed for 7.5 h, cooled, and poured into about 500 mL of ice-cold 10% (w/w) aqueous HCl. The gray precipitate was collected by suction filtration, washed with about 500 mL of water, and dried to give about 25.5 g of crude ix. This material was then dissolved in about 500 mL of diethyl ether, dried over MgSO<sub>4</sub>, filtered, concentrated, and crystallized. This material was then triturated with about 100 mL of hot diethyl ether, cooled, diluted with about 100 mL hexane, and the solid was then collected by suction filtration to give about 20.3 g of beige powder, ix. This material (20.3 g, 39.6 mmol) was dissolved in about 80 mL of dry THF (tetrahydrofuran) under argon at room temperature, and about 5.5 mL (43 mmol) of N,N-dimethylaniline was added. The stirred mixture was cooled in an ice water bath and a solution of acryloyl chloride (3.5 mL, 43 mmol) in dry THF (20 mL) was added over 5 minutes by dropping funnel. The bath was removed and the mixture was stirred at room temperature for 20 h. The mixture was then slowly poured into a vigorously stirred mixture of crushed ice (about 300 mL) and 25% HCl (about 200 mL). The greenish white solid was collected by suction filtration and dried under vacuum. This material was then purified by flash chromatography over silica gel, using ethyl acetate and ligroin mixtures to elute fractions. About 17.3 g of the desired monomer, M1, was obtained as a beige glass upon solvent removal.



About 5.66 g (0.01 mol) of monomer M1, about 4.33 g (0.03 mol) of 2-ethoxyethyl acrylate, about 0.41 g (0.002 mol) of 2-acrylamido-2-methyl propanoic acid, and about 40 mL of DMF (dimethyl formamide) were 25 mixed in a 100 mL 3-neck round bottom flask equipped with a nitrogen inlet, a mechanical stirrer, and a condenser. The flask was immersed in a constant temperature bath at 80° C. and purged with nitrogen for 30 minutes. About 0.26 g of AIBN (2,2'-azobis[2-methyl 30 propionitrile]) in about 2 mL of DMF was added to initiate polymerization. After about 4 h about 0.13 g of additional AIBN was added. The polymerization was allowed to proceed at 80° C. for an additional 16 h. The polymer solution was diluted with about 150 mL of acetone and dispersed in about 900 mL of hot distilled water with agitation. A milky polymer dispersion of M2 was obtained. This dispersion was dialyzed against distilled water overnight and concentrated to 6.31% solids with an Amicon diafiltration unit. The z-average particle size measured with a Malvern Autosizer IIC was about 180 nm. The elemental analysis results were: C (45.74%); H (4.73%); N (6.21%); Cl (8.6%).



About 95 g of M3 were dissolved in about 28.5 g of ethyl acetate at about 60° C. An aqueous gelatin solution comprising about 3.8 g of 10% (w/w) Alkanol-XC, about 22.8 g 12.5% (w/w) aqueous gelatin, and about 30.4 g water was prepared. These aqueous and ethyl acetate solutions were then combined with stirring and passed through a colloid mill five times to obtain a fine particle dispersion of M3. The resulting dispersion was chill set, noodled, and washed for about 4 h to remove

the ethyl acetate. This dispersion was then remelted, chill set, and stored until use.

#### Preparation of Test Coatings

A test coating structure and format nearly identical to that described above for Examples 1 and 2 was utilized. The same coating support and receiver were utilized. Polymeric coupler M2 (1035 mg/m<sup>2</sup>; Example 11) was coated at a molar equivalent of coupling sites, relative to the coated level of M3 (687 mg/m<sup>2</sup>) in Example 10. Blue sensitized silver chloride at a coverage of about 537 mg/m<sup>2</sup> was coated with polymeric coupler M2. Green sensitized silver chloride at a coverage of about 408 mg/m<sup>2</sup> was coated with coupler M3. A thermal solvent dispersion of p-hydroxy-2-ethylhexyl benzoate, prepared as described earlier, was used, and this thermal solvent was coated at a level of 687 mg/m<sup>2</sup> in the dye forming layer. Gelatin was coated at about 687 mg/m<sup>2</sup> in the light sensitive layers. The second (overcoat) layers, and the same proportion of hardener, MBSE, were coated identically as described earlier for Examples 1 and 2.

#### Evaluation

Several sets of these coatings were exposed and processed as described above for Examples 1 and 2; the same wet development solution, stop bath, buffer bath, and wash sequence were used. Thermal transfer was then activated by passing these test coatings through the heated pinch rollers at 110° C. ten times as earlier described. The silver halide and dye forming layer and overcoat were removed using the adhesion sheet stripping method described above. HPLC analysis of the D<sub>min</sub> and D<sub>max</sub> regions of the receiver elements from these coatings for transferred dye is illustrated in Table 5. The coating of the present invention, containing the polymeric magenta coupler M2 (Example 11), yielded substantially more transferred dye (32.4%) than the comparison coating of M3 (Example 10).

The invention has been described in detail with particular reference to preferred embodiments thereof, but it will be understood that variations and modifications can be effected within the spirit and scope of the invention.

TABLE 5

| Magenta Dyes Transferred to Receiver     |                  |                                      |
|------------------------------------------|------------------|--------------------------------------|
| Coating                                  | Region           | Dye in Receiver (mg/m <sup>2</sup> ) |
| Example 10<br>(Comparison; M3)           | D <sub>min</sub> | 0.2                                  |
| Example 11<br>(Present Invention;<br>M2) | D <sub>max</sub> | 17.9                                 |
|                                          | D <sub>min</sub> | 0.1                                  |
|                                          | D <sub>max</sub> | 23.7                                 |

What is claimed is:

1. A process for forming a dye image comprising the steps of: exposing a photographic element comprising one and only one support bearing a light sensitive silver halide emulsion layer containing a polymeric color coupler compound capable of forming a heat transferable dye upon development, wherein the polymeric color coupler compound is of the formula:

COUP-L-B

wherein COUP represents a coupler moiety capable of forming a heat transferable dye upon reaction of the

moiety with an oxidation product of a color developer; L is a divalent linking group which is separated from COUP upon reaction of the coupler moiety with said oxidation product of a color developer; and B represents the polymeric backbone;

developing said exposed element in an external color developer solution to form a heat transferable dye image;

stopping said development with an acid stop bath; heating said exposed, developed element to thereby transfer the dye image from the emulsion layer to a dye receiving layer, wherein said receiving layer is part of the photographic element or part of a separate dye receiving element brought into contact with the photographic element; and

separating the emulsion layer from the dye receiving layer containing the transferred dye image.

2. The process of claim 1, wherein said color developer solution comprises a p-phenylenediamine.

3. The process of claim 2, wherein said color developer solution comprises 4-amino-N,N-diethylaniline hydrochloride; 4-amino-3-methyl-N,N-diethylaniline hydrochloride; 4-amino-3-methyl-N-ethyl-N-( $\beta$ -methanesulfonamidoethyl)aniline sulfate hydrate; 4-amino-3-methyl-N-ethyl-N-( $\beta$ -hydroxyethyl)aniline sulfate; 4-amino-3-( $\beta$ -methanesulfonamido)ethyl-N,N-diethylaniline hydrochloride; 4-amino-3-methyl-N-ethyl-N-( $\beta$ -methanesulfonamidoethyl)aniline sesquisulfate monohydrate; or 4-amino-3-methyl-N-ethyl-N-(2-methoxyethyl)aniline di-p-toluenesulfonic acid.

4. The process of claim 1 wherein said dye receiving layer comprises polycarbonate, polyurethane, polyester, polyvinyl chloride, poly(styrene-coacrylonitrile), poly(caprolactone) or mixtures thereof.

5. The process of claim 1 wherein said dye receiving layer is an integral layer of said photographic element.

6. The process of claim 5, wherein said dye receiving layer is present between the support and the emulsion layer of the photographic element, and wherein after the dye image is transferred from the emulsion layer to the dye receiving layer, the emulsion layer is separated from the dye receiving layer.

7. The process of claim 1, wherein said dye receiving layer is contained in a separate dye receiving element, and further comprising the step of bringing together the dye receiving element and the photographic element prior to or during heating step (c).

8. The process of claim 1, wherein said heating step comprises exposing the photographic element to a temperature of from 50° C. to 200° C. for from 10 seconds to 30 minutes.

9. The process of claim 8, wherein said heating step comprises exposing the photographic element to a temperature of from 75° C. to 160° C. for from 10 seconds to 30 minutes.

10. The process of claim 9, wherein said heating step comprises exposing the photographic element to a temperature of from 80° C. to 120° C. for from 10 seconds to 30 minutes.

11. The process of claim 1, wherein said heating step comprises running said photographic element and said receiving layer through rollers at a temperature of 75° C. to 190° C., a pressure of 500 Pa to 1,000 kPa, and a speed of 0.1 cm/s to 50 cm/s.

12. The process of claim 1, wherein said COUP moiety is of the phenol type (formula C-I) or the naphthol type (formulae C-II and C-III) or of the type C-IV as presented in the formulae below; wherein the asterisk

mark indicates the position of the bond to said divalent linking group L;



and wherein

$R_1$  has 0 to 30 carbon atoms and represents a possible 35 substituent on the phenol ring or naphthol ring;

$R_2$  represents  $-\text{CONR}_3\text{R}_4$ ,  $-\text{NHCOR}_3$ ,  $-\text{NHCOOR}_5$ ,  $-\text{NHSO}_2\text{R}_5$ ,  $-\text{NHCONR}_3\text{R}_4$ , or  $-\text{NHSO}_2\text{R}_3\text{R}_4$ ,  $\text{R}_3$  and  $\text{R}_4$  each independently represents a hydrogen atom, aliphatic group having 1 to 30 carbon atoms, aromatic group having from 6 to 30 carbon atoms, or heterocyclic group having from 2 to 30 carbon atoms;

R<sub>5</sub> represents an aliphatic group having from 1 to 30 carbon atoms, aromatic group having from 6 to 30 carbon atoms, or heterocyclic group;

**R<sub>3</sub>** and **R<sub>4</sub>** may join each other to form a heterocyclic ring; p is an integer from 0 to 3; q and r are integers from 0 to 4; s is an integer from 0 to 2;

$X_1$  represents an oxygen atom, sulfur atom, or  $R_6N <-$  group, where  $R_6$  represents a hydrogen atom, an aliphatic group having from 1 to 30 carbon atoms, an aromatic group having from 6 to 30 carbon atoms, a heterocyclic group having from 2 to 30 carbon atoms, a carbonamido group having from 1 to 30 carbon atoms, an imido group having from 4 to 30 carbon atoms,  $-OR_7$ ,  $-SR_7$ ,  $-COR_7$ ,  $-CONR_7R_8$ ,  $-COCOR_7$ ,  $-COCOR_7R_8$ ,  $-COOR_7$ ,  $-COCOOR_9$ ,  $-SO_2R_9$ ,  $-SO_2OR_9$ ,  $-SO_2NR_7R_8$ , or  $-NR_7R_8$ ; where  $R_7$  and  $R_8$  each independently represent a hydrogen atom, an aliphatic group having from 1 to 30 carbon atoms, an aromatic group having from 6 to 30 carbon atoms, or a heterocyclic group having from 2 to 30 carbon atoms;  $R_7$  and  $R_8$  may join each other to form a heterocyclic ring;  $R_9$  represent an aliphatic group having from 1 to 30 carbon atoms, an aromatic

group having from 6 to 30 carbon atoms, or a heterocyclic group having from 2 to 30 carbon atoms; T represents a group of atoms required to form a 5-, 6-, or 7-membered ring, wherein T is



or a combination thereof, and wherein R' and R" each independently represents a hydrogen atom, alkyl group, aryl group, halogen atom, alkyloxy group, alkyloxycarbonyl group, arylcarbonyl group, alkylcarbamoyl group, arylcarbamoyl group or cyano group.

C-III      group, alkylcarbamoyl group, arylcarbamoyl group or cyano group.

20      13. The process of claim 12, wherein said R<sub>1</sub> is selected from the group comprising an alkyl group, an alkenyl group, an alkoxy group, an alkoxy carbonyl group, a halogen atom, an alkoxy carbamoyl group, an aliphatic amido group, an alkylsulfamoyl group, an alkylsulfonamido group, an alkylureido group, an arylcarbamoyl group, an arylamido group, an arylsulfamoyl group, an arylsulfonamido group, an arylureido group, hydroxyl group, amino group, carboxyl group, sulfo group, heterocyclic group, carbonamido group, sulfonamido group, carbamoyl group, sulfamoyl group, ureido group, acyloxy group, aliphatic oxy group, aliphatic thio group, aliphatic sulfonyl group, aromatic oxy group, aromatic thio group, aromatic sulfonyl group, sulfamoyl amino group, nitro group, and imido group.

C-IV

25

30

35

40 14. The process of claim 12, wherein said R<sub>3</sub> and R<sub>4</sub> are each independently selected from the group comprising a hydrogen atom, methyl, ethyl, butyl, methoxyethyl, n-decyl, n-dodecyl, n-hexadecyl, trifluoromethyl, heptafluoropropyl, dodecyloxypropyl, 2,4-di-t-amylphenoxy-propyl, 2,4-di-t-amylphenoxybutyl, phenyl, tolyl, 2-tetradecyloxyphenyl, pentafluorophenyl, and 45 2-chloro-5-dodecyloxy carbonyl phenyl, 2-pyridyl, 4-pyridyl, 2-furyl, and 2-thienyl.

50 15. The process of claim 12, wherein said R<sub>5</sub> is selected from the group comprising methyl, ethyl, butyl, methoxyethyl, n-decyl, n-dodecyl, and n-hexadecyl, phenyl, tolyl, 4-chlorophenyl, naphthyl, 2-pyridyl, 4-pyridyl, and 2-furyl.

16. The process of claim 12, wherein said R<sub>3</sub> and R<sub>4</sub> may join each other to form a heterocyclic ring selected from the group comprising a morpholine ring, a piperidine ring, and a pyrrolidine ring.

17. The process of claim 12, wherein said R<sub>6</sub> is selected from the group comprising methyl, ethyl, butyl, methoxyethyl, benzyl, phenyl, tolyl, 2-pyridyl and 2-pyrimidyl, formamido, acetamido, N-methylacetamido, toluenesulfonamido, and 4-chlorobenzenesulfonamido, succinimido.

18. The process of claim 12, wherein said R<sub>7</sub>, R<sub>8</sub> and R<sub>9</sub> may independently be selected from the group comprising methyl, ethyl, butyl, methoxyethyl, n-decyl, 65 n-dodecyl, n-hexadecyl, trifluoromethyl, heptafluoropropyl, dodecyloxypropyl, 2,4-di-t-amylphenoxypropyl, 2,4-di-t-amylphenoxybutyl, phenyl, tolyl, 2-tetradecyloxy phenyl, pentafluorophenyl, and 2-chloro-5-

dodecyloxycarbonylphenyl, 2-pyridyl, 4-pyridyl, 2-furyl, and 2-thienyl.

19. The process of claim 12, wherein said R<sub>7</sub> and R<sub>8</sub> may join each other to form a heterocyclic ring selected from the group comprising a morpholine ring, a piperidine ring, and a pyrrolidine ring.

20. The process of claim 1, wherein said COUP moiety is of the pyrazolotriazole-type and imidazopyrazole-type (formulae M-I to M-VII presented below); the asterisk mark indicates the position of the bond to said 10 divalent linking group L;



wherein

R<sub>1</sub> and R<sub>2</sub> each independently represents a substituent selected from the group comprising alkyl, substituted alkyl, an aryl, substituted aryl, alkoxy, aryloxy, alkoxy carbonyl, acylamino, carbamoyl, alkyl carbamoyl group, dialkyl carbamoyl, aryl carbamoyl, alkylsulfonyl, arylsulfonyl, alkylsulfonamido, arylsulfonamido, sulfamoyl, alkylsulfamoyl, dialkylsulfamoyl, arylsulfamoyl, alkylthio group, arylthio, cyano, nitro, and a halogen atom;

R<sub>3</sub>, R<sub>4</sub>, R<sub>5</sub>, and R<sub>6</sub> are each independently selected from the group comprising hydrogen atom, hydroxyl group, unsubstituted alkyl, substituted alkyl, aryl, heterocyclic, alkylamino, acylamino, anilino, alkoxy carbonyl, alkyl carbonyl, aryl carbonyl, alkylthio, arylthio, carbamoyl, sulfamoyl, and alkyl sulfonamido.

21. The process of claim 20, wherein R<sub>1</sub> and R<sub>2</sub> each independently is selected from the group comprising halo-alkyl, cyano-alkyl, benzyl-alkyl, methyl-aryl, ethyl-aryl, methoxy, ethoxy, phenoxy, methoxy carbonyl, acetylamino, methylcarbamoyl, ethylcarbamoyl, dimethylcarbamoyl, phenylcarbamoyl, methylsulfonyl, phenylsulfonyl, methanesulfonamido, phenylsulfonamido, ethylsulfamoyl, dimethylsulfamoyl, meth-

ylthio, phenylthio, fluorine atom, chlorine atom, and bromine atom.

22. The process of claim 20, wherein R<sub>3</sub>, R<sub>4</sub>, R<sub>5</sub>, and R<sub>6</sub> are each independently selected from the group comprising methyl, propyl, t-butyl, trifluoromethyl, tridecyl, phenyl, 4-t-butylphenyl, 2,4-di-t-amylphenyl, 4-methoxyphenyl, 2-furyl, 2-thienyl, 2-pyrimidinyl, 2-benzthiazolyl, methylamino, diethylamino, t-butylamino, acetylamino, propylamido, benzamido, phenylamino, 2-chloroanilino, methoxycarbonyl, butoxycarbonyl, 2-ethylhexyloxycarbonyl, acetyl, butylcarbonyl, cyclohexylcarbonyl, benzoyl, 4-t-butylbenzoyl, methylthio, octylthio, 2-phenoxyethylthio, phenylthio, 2-butoxy-5-t-octylphenylthio, N-ethylcarbamoyl, N,N-dibutylcarbamoyl, N-methyl-N-butylcarbamoyl, N-ethylsulfamoyl, N,N-diethylsulfamoyl, N,N-dipropylsulfamoyl, benzenesulfonamido, and p-toluenesulfonamido.

23. The process of claim 1, wherein said photographic element further comprises a layer containing a thermal solvent.

24. An aqueous alkaline developable photographic element comprising one and only one support bearing a light sensitive silver halide emulsion layer, a layer containing a polymeric color coupler compound capable of forming a heat transferable dye upon development in an external alkaline color developer solution, a layer containing a thermal solvent for facilitating the diffusion of said dye, said layers further comprising a hydrophilic colloid, and further bearing between said support and said light sensitive layer a polymeric receive layer capable of absorbing said heat transferable dye upon thermal activation and diffusion of said dye, wherein said polymeric color coupler compound is of the formula:

#### COUP-L-B

wherein COUP represents a coupler moiety capable of forming a heat transferable dye upon reaction of the moiety with the oxidation product of a color developing agent; L is a divalent linking group which is separated from COUP upon reaction of the coupler moiety with said oxidation product of said color developing agent; and B represents the polymeric backbone.

25. The element of claim 24, wherein said COUP moiety is of the phenol type (formula C-I) or the naphthol type (formulae C-II and C-III) or of the type C-IV as presented in the formulae below; wherein the asterisk mark indicates the position of the bond to said divalent linking group L;





and wherein

R<sub>1</sub> has 0 to 30 carbon atoms and represents a possible substituent on the phenol ring or naphthol ring;

R<sub>2</sub> represents —CONR<sub>3</sub>R<sub>4</sub>, —NHCOR<sub>3</sub>, —NHCOOR<sub>5</sub>, —NHSO<sub>2</sub>R<sub>5</sub>, —NHCONR<sub>3</sub>R<sub>4</sub>, or —NHSO<sub>2</sub>R<sub>3</sub>R<sub>4</sub>, R<sub>3</sub> and R<sub>4</sub> each independently represents a hydrogen atom, aliphatic group having 1 to 30 carbon atoms, aromatic group having from 6 to 30 carbon atoms, or heterocyclic group having from 2 to 30 carbon atoms;

R<sub>5</sub> represents an aliphatic group having from 1 to 30 carbon atoms, aromatic group having from 6 to 30 carbon atoms, or heterocyclic group;

R<sub>3</sub> and R<sub>4</sub> may join each other to form a heterocyclic ring; p is an integer from 0 to 3; q and r are integers from 0 to 4; s is an integer from 0 to 2;

X<sub>1</sub> represents an oxygen atom, sulfur atom, or R<sub>6</sub>N<-group, where R<sub>6</sub> represents a hydrogen atom, an aliphatic group having from 1 to 30 carbon atoms, an aromatic group having from 6 to 30 carbon atoms, a heterocyclic group having from 2 to 30 carbon atoms, a carbonamido group having from 1 to 30 carbon atoms, an imido group having from 4 to 30 carbon atoms, —OR<sub>7</sub>, —SR<sub>7</sub>, —COR<sub>7</sub>, —CONR<sub>7</sub>R<sub>8</sub>, —COCOR<sub>7</sub>, —COCOR<sub>7</sub>R<sub>8</sub>, —COOR<sub>7</sub>, —COCOOR<sub>9</sub>, —SO<sub>2</sub>R<sub>9</sub>, —SO<sub>2</sub>OR<sub>9</sub>, —SO<sub>2</sub>NR<sub>7</sub>R<sub>8</sub>, or —NR<sub>7</sub>R<sub>8</sub>; where R<sub>7</sub> and R<sub>8</sub> each independently represent a hydrogen atom, an aliphatic group having from 1 to 30 carbon atoms, an aromatic group having from 6 to 30 carbon atoms, or a heterocyclic group having from 2 to 30 carbon atoms; R<sub>7</sub> and R<sub>8</sub> may join each other to form a heterocyclic ring; R<sub>9</sub> represents an aliphatic group having from 1 to 30 carbon atoms, an aromatic group having from 6 to 30 carbon atoms, or a heterocyclic group having from 2 to 30 carbon atoms;

T represents a group of atoms required to form a 5-, 6-, or 7-membered ring, wherein T is



or a combination thereof, and wherein R' and R'' each independently represents a hydrogen atom,

alkyl group, aryl group, halogen atom, alkyloxy group, alkyloxycarbonyl group, arylcarbonyl group, alkylcarbamoyl group, arylcarbamoyl group or cyano group.

5 26. The element of claim 25, wherein said R<sub>1</sub> is selected from the group comprising an alkyl group, an alkenyl group, an alkoxy group, an alkoxy carbonyl group, a halogen atom, an alkoxy carbonyl group, an 10 aliphatic amido group, an alkylsulfamoyl group, an alkylsulfamido group, an alkylureido group, an arylcarbamoyl group, an arylamido group, an arylsulfamoyl group, an arylsulfamido group, an arylureido group, hydroxyl group, amino group, carboxyl group, sulfo group, heterocyclic group, carbonamido group, sulfonamido group, carbamoyl group, sulfamoyl group, ureido group, acyloxy group, aliphatic oxy group, aliphatic thio group, aliphatic sulfonyl group, aromatic 15 oxy group, aromatic thio group, aromatic sulfonyl group, sulfamoyl amino group, nitro group, and imido group.

27. The element of claim 25, wherein said R<sub>3</sub> and R<sub>4</sub> are each independently selected from the group comprising a hydrogen atom, methyl, ethyl, butyl, methoxyethyl, n-decyl, n-dodecyl, n-hexadecyl, trifluoromethyl, heptafluoropropyl, dodecyloxypropyl, 2,4-di-t-amylphenoxy-propyl, 2,4-di-t-amylphenoxybutyl, phenyl, tolyl, 2-tetradecyloxyphenyl, pentafluorophenyl, and 2-chloro-5-dodecyloxycarbonyl phenyl, 2-pyridyl, 4-pyridyl, 2-furyl, and 2-thienyl.

28. The element of claim 25, wherein said R<sub>5</sub> is selected from the group comprising methyl, ethyl, butyl, methoxyethyl, n-decyl, n-dodecyl, and n-hexadecyl, phenyl, tolyl, 4-chlorophenyl, naphthyl, 2-pyridyl, 4-pyridyl, and 2-furyl.

29. The element of claim 25, wherein said R<sub>3</sub> and R<sub>4</sub> may join each other to form a heterocyclic ring selected from the group comprising a morpholine ring, a piperidine ring, and a pyrrolidine ring.

30. The element of claim 25, wherein said R<sub>6</sub> is selected from the group comprising methyl, ethyl, butyl, methoxyethyl, benzyl, phenyl, tolyl, 2-pyridyl and 2-pyrimidyl, formamido, acetamido, N-methylacetamido, toluenesulfonamido, and 4-chlorobenzenesulfonamido, succinimido.

31. The element of claim 25, wherein said R<sub>7</sub>, R<sub>8</sub> and R<sub>9</sub> may independently be selected from the group comprising methyl, ethyl, butyl, methoxyethyl, n-decyl, n-dodecyl, n-hexadecyl, trifluoromethyl, heptafluoropropyl, dodecyloxypropyl, 2,4-di-t-amylphenoxypropyl, 2,4-di-t-amylphenoxybutyl, phenyl, tolyl, 2-tetradecyloxyphenyl, pentafluorophenyl, and 2-chloro-5-dodecyloxycarbonylphenyl, 2-pyridyl, 4-pyridyl, 2-furyl, and 2-thienyl.

32. The element of claim 25, wherein said R<sub>7</sub> and R<sub>8</sub> may join each other to form a heterocyclic ring selected from the group comprising a morpholine ring, a piperidine ring, and a pyrrolidine ring.

33. The element of claim 25, wherein said COUP moiety is of the pyrazolotriazole-type and imidazopyrazole-type (formulae M-I to M-VII presented below); the asterisk mark indicates the position of the bond to said divalent linking group L;



wherein

R<sub>1</sub> and R<sub>2</sub> each independently represents a substituent selected from the group comprising alkyl, substituted alkyl, an aryl, substituted aryl, alkoxy, aryloxy, alkoxy carbonyl, acylamino, carbamoyl, alkyl carbamoyl group, dialkyl carbamoyl, aryl carbamoyl, alkylsulfonyl, arylsulfonyl, alkylsulfonamido, arylsulfonamido, sulfamoyl, alkylsulfamoyl, dialkylsulfamoyl, arylsulfamoyl, alkylthio group, arylthio, cyano, nitro, and a halogen atom; R<sub>3</sub>, R<sub>4</sub>, R<sub>5</sub>, and R<sub>6</sub> are each independently selected from the group comprising hydrogen atom, hydroxyl group, unsubstituted alkyl, substituted alkyl, aryl, heterocyclic, alkylamino, acylamino, anilino, alkoxy carbonyl, alkyl carbonyl, aryl carbonyl, alkylthio, arylthio, carbamoyl, sulfamoyl, and alkyl sulfonamido.

34. The element of claim 33, wherein R<sub>1</sub> and R<sub>2</sub> each independently is selected from the group comprising halo-alkyl, cyano-alkyl, benzyl-alkyl, methyl-aryl, ethyl-aryl, methoxy, ethoxy, phenoxy, methoxy carbonyl, acetyl amino, methyl carbamoyl, ethyl carbamoyl, dimethyl carbamoyl, phenyl carbamoyl, methylsulfonyl, phenylsulfonyl, methanesulfonamido, phenylsulfonamido, ethylsulfamoyl, dimethylsulfamoyl, methythio, phenylthio, fluorine atom, chlorine atom, and bromine atom.

35. The element of claim 34, wherein R<sub>3</sub>, R<sub>4</sub>, R<sub>5</sub>, and R<sub>6</sub> are each independently selected from the group comprising methyl, propyl, t-butyl, trifluoromethyl, tridecyl, phenyl, 4-t-butylphenyl, 2,4-di-t-amylphenyl, 4-methoxyphenyl, 2-furyl, 2-thienyl, 2-pyrimidinyl, 2-benzthiazolyl, methylamino, diethylamino, t-butylamino, acetyl amino, propylamido, benzamido, phenylamino, 2-chloroanilino, methoxycarbonyl, butoxycarbonyl, 2-ethylhexyloxycarbonyl, acetyl,

butyl carbonyl, cyclohexyl carbonyl, benzoyl, 4-t-butylbenzoyl, methylthio, octylthio, 2-phenoxyethylthio, phenylthio, 2-butoxy-5-t-octylphenylthio, N-ethyl carbamoyl, N,N-dibutyl carbamoyl, N-methyl-N-butyl carbamoyl, N-ethylsulfamoyl, N,N-diethylsulfamoyl, N,N-dipropylsulfamoyl, benzenesulfonamido, and p-toluenesulfonamido.

36. The element of claim 24, wherein said hydrophilic colloid comprises gelatin, polyvinyl alcohol, or polyvinylpyrrolidone.

37. The element of claim 36, wherein said hydrophilic colloid is gelatin.

38. The element of claim 24, wherein said solvent is a phenol derivative.

39. The element of claim 38, wherein said thermal solvent is incorporated in a given layer in an amount of 1-300 % by weight of the total amount of hydrophilic binder incorporated in said layer.

40. The element of claim 24, wherein said polymeric receiver layer comprises polymer selected from the group comprising polycarbonates, polyurethanes, polyesters, polyvinyl chlorides, poly(styrene-co-acrylonitrile)s, poly(caprolactone)s and mixtures thereof.

41. The process of claim 1, wherein said COUP moiety is of the acylacetanilide type (formula Y-I) and benzoylacetanilide type (Formulae Y-II and Y-III) as presented below; the asterisk mark indicates the position of the bond to said divalent linking group L;



wherein

R<sub>1</sub>, R<sub>2</sub>, R<sub>3</sub>, R<sub>4</sub>, and R<sub>5</sub> each independently are selected from the group comprising a hydrogen atom, an alkyl group, an alkenyl group, an alkoxy group, an alkoxy carbonyl group, a halogen atom, an alkoxy carbamoyl group, an aliphatic amido group, an alkylsulfamoyl group, an alkylsulfonamido group, an alkylureido group, an alkyl-substituted succinimido group, an aryloxy group, an aryloxycarbonyl group, an aryl carbamoyl group, an arylamido group, an arylsulfamoyl group, an arylsulfonamido group, an arylureido group, carboxyl group, sulfo group, nitro group, cyano group, and thiocyanato group.

42. The element of claim 24, wherein said COUP moiety is of the acylacetanilide type (formula Y-I) and benzoylacetanilide type (Formulae Y-II and Y-III) as presented below; the asterisk mark indicates the position of the bond to said divalent linking group L;



wherein

R<sub>1</sub>, R<sub>2</sub>, R<sub>3</sub>, R<sub>4</sub>, and R<sub>5</sub> each independently are selected from the group comprising a hydrogen atom, an alkyl group, an alkenyl group, an alkoxy group, an alkoxy carbonyl group, a halogen atom, an alkoxy carbamoyl group, an aliphatic amido group, an alkylsulfamoyl group, an alkylsulfonamido group, an alkylureido group, an alkyl-substituted succinimido group, an aryloxy group, an aryloxy carbonyl group, an arylcarbamoyl group, an arylamido group, an arylsulfamoyl group, an arylsulfonamido group, an arylureido group, carboxyl group, sulfo group, nitro group, cyano group, and thiocyanato group.

43. A process for forming a dye image comprising the steps of:

exposing a photographic element comprising one and only one support bearing a light sensitive silver halide emulsion layer containing a polymeric color coupler compound capable of forming a heat transferable dye upon development, wherein the polymeric color coupler compound is of the formula:

COUP-L-B

wherein COUP represents a coupler moiety capable of forming a heat transferable dye upon reaction of the moiety with an oxidation product of a color developer; L is a divalent linking group which is separated from COUP upon reaction of the coupler moiety with said oxidation product of a

55

- color developer; and B represents the polymeric backbone;
- 5 developing said exposed element in an external aqueous alkaline color developer solution to form a heat transferable dye image;
- 10 heating said exposed, developed element to thereby transfer the dye image from the emulsion layer to a dye receiving layer, where said receiving layer is part of the photographic element or part of a separate dye receiving element brought into contact with the photographic element; and
- 15 separating the emulsion layer from the dye receiving layer containing the transferred dye image, and wherein
- 20 bleaching, fixing, and bleach-fixing steps after the development step are excluded.
44. The process of claim 43, wherein said color developer solution comprises a p-phenylenediamine.
45. The process of claim 43 wherein said dye receiving layer comprises polycarbonate, polyurethane, polyether, polyvinyl chloride, poly(styrene-coacrylonitrile), poly(caprolactone) or mixtures thereof.
46. The process of claim 43 wherein said dye receiving layer is an integral layer of said photographic element.
47. The process of claim 43, wherein said dye receiving layer is present between the support and the emulsion layer of the photographic element, and wherein after the dye image is transferred from the emulsion layer to the dye receiving layer, the emulsion layer is separated from the dye receiving layer.
48. The process of claim 43, wherein said dye receiving layer is contained in a separate dye receiving element, and further comprising the step of bringing together the dye receiving element and the photographic element prior to or during heating step.
49. The process of claim 43, wherein said heating step comprises exposing the photographic element to a temperature of from 75° C. to 160° C. for from 10 seconds to 30 minutes.
50. The process of claim 43, wherein said heating step comprises exposing the photographic element to a temperature of from 80° C. to 120° C. for from 10 seconds to 30 minutes.
51. The process of claim 43, wherein said heating step comprises running said photographic element and said receiving layer through rollers at a temperature of 75° C. to 190° C., a pressure of 500 Pa to 1,000 kPa, and a speed of 0.1 cm/s to 50 cm/s.
52. The process of claim 43, wherein said photographic element further comprises a thermal solvent.
53. The process of claim 43, further comprising the step of stopping said development with an acid stop bath after development and before the heating step.

\* \* \* \* \*

UNITED STATES PATENT AND TRADEMARK OFFICE  
CERTIFICATE OF CORRECTION

PATENT NO. : **5,354,642**

Page 1 of 3

DATED : **October 11, 1994**

INVENTOR(S) : **John Texter et al.**

It is certified that error appears in the above-identified patent and that said Letters Patent is hereby corrected as shown below:

Column 57, line 30,



should read --



Column 59, line 22,



should read --



Column 59, line 30



should read --



UNITED STATES PATENT AND TRADEMARK OFFICE  
CERTIFICATE OF CORRECTION

PATENT NO. : **5,354,642**

Page 2 of 3

DATED : **October 11, 1994**

INVENTOR(S) : **John Texter et al.**

It is certified that error appears in the above-identified patent and that said Letters Patent is hereby corrected as shown below:

Column 59, line 37



should read



Column 60, line 36, --receive-- should read "receiver".

Column 61, line 5



should read



UNITED STATES PATENT AND TRADEMARK OFFICE  
CERTIFICATE OF CORRECTION

PATENT NO. : **5,354,642**  
DATED : **October 11, 1994**  
INVENTOR(S) : **John Texter et al.**

Page 3 of 3

It is certified that error appears in the above-identified patent and that said Letters Patent is hereby corrected as shown below:

Column 61, line 15,



should read --



Signed and Sealed this  
Eighteenth Day of July, 1995

Attest:



BRUCE LEHMAN

Attesting Officer

Commissioner of Patents and Trademarks